



US007371491B2

(12) **United States Patent**  
Niimi et al.

(10) **Patent No.:** US 7,371,491 B2  
(45) **Date of Patent:** May 13, 2008

(54) **ELECTROPHOTOGRAPHIC PHOTORECEPTOR, METHOD FOR MANUFACTURING THE ELECTROPHOTOGRAPHIC PHOTORECEPTOR, AND IMAGE FORMING APPARATUS AND PROCESS CARTRIDGE USING THE ELECTROPHOTOGRAPHIC PHOTORECEPTOR**

(75) Inventors: **Tatsuya Niimi**, Numazu (JP); **Nozomu Tamoto**, Numazu (JP); **Katsuichi Ohta**, Mishima (JP)

(73) Assignee: **Ricoh Company Limited**, Tokyo (JP)

(\*) Notice: Subject to any disclaimer, the term of this patent is extended or adjusted under 35 U.S.C. 154(b) by 422 days.

(21) Appl. No.: 10/944,614

(22) Filed: Sep. 20, 2004

(65) **Prior Publication Data**

US 2005/0069797 A1 Mar. 31, 2005

(30) **Foreign Application Priority Data**

Sep. 30, 2003 (JP) ..... 2003-342515  
Dec. 1, 2003 (JP) ..... 2003-401588

(51) **Int. Cl.**

G03G 5/047 (2006.01)  
G03G 5/14 (2006.01)

(52) **U.S. Cl.** ..... 430/59.5; 430/65; 430/60;  
430/131; 430/133; 430/134; 399/159

(58) **Field of Classification Search** ..... 430/64,  
430/65, 66, 59.5, 131, 133, 134; 399/159  
See application file for complete search history.

(56) **References Cited**

U.S. PATENT DOCUMENTS

5,215,839 A 6/1993 Yu

5,576,131 A \* 11/1996 Takai et al. ..... 430/59.2  
5,677,096 A \* 10/1997 Suzuki ..... 430/58.75  
6,132,911 A 10/2000 Niimi  
6,218,533 B1 4/2001 Niimi  
6,268,096 B1 7/2001 Nukada et al.

(Continued)

FOREIGN PATENT DOCUMENTS

EP 1 081 557 A1 3/2001

(Continued)

OTHER PUBLICATIONS

U.S. Appl. No. 11/068,180, filed Mar. 1, 2005, Tamoto et al.

(Continued)

Primary Examiner—Christopher RoDee

(74) Attorney, Agent, or Firm—Oblon, Spivak, McClelland, Maier & Neustadt, P.C.

(57) **ABSTRACT**

A photoreceptor including an electroconductive substrate; and a charge blocking layer; a moiré preventing layer; and a photosensitive layer, which are overlaid overlying the substrate in this order, wherein the photosensitive layer includes a titanyl phthalocyanine crystal which has an average primary particle diameter not greater than 0.25  $\mu$ m, and has an X-ray diffraction spectrum such that a maximum peak is observed at a Bragg (20) angle of  $27.2^\circ \pm 0.2^\circ$ ; a peak is observed at Bragg (20) angle of  $9.4^\circ \pm 0.2^\circ$ ,  $9.6 \pm 0.2^\circ$  and  $24.0 \pm 0.2^\circ$ ; a lowest angle peak is observed at an angle of  $7.3^\circ \pm 0.2^\circ$ ; no peak is observed between the lowest angle peak and the  $9.4^\circ$  peak; and no peak is observed at a Bragg (20) angle of  $26.3^\circ \pm 0.2^\circ$ , when a Cu—K $\alpha$  X-ray having a wavelength of 0.1542 nm (1.542  $\text{\AA}$ ) is used.

28 Claims, 15 Drawing Sheets



## U.S. PATENT DOCUMENTS

|              |      |         |                     |         |
|--------------|------|---------|---------------------|---------|
| 6,369,842    | B1 * | 4/2002  | Abramsohn .....     | 430/127 |
| 6,558,863    | B2   | 5/2003  | Rokutanzono et al.  |         |
| 6,677,091    | B2   | 1/2004  | Niimi               |         |
| 2003/0113642 | A1   | 6/2003  | Kami et al.         |         |
| 2004/0033428 | A1   | 2/2004  | Niimi               |         |
| 2004/0053149 | A1   | 3/2004  | Toda et al.         |         |
| 2004/0120730 | A1   | 6/2004  | Niimi et al.        |         |
| 2004/0126686 | A1   | 7/2004  | Toda et al.         |         |
| 2004/0253527 | A1 * | 12/2004 | Suzuki et al. ..... | 430/66  |

## FOREIGN PATENT DOCUMENTS

|    |           |         |
|----|-----------|---------|
| JP | 61-239248 | 10/1986 |
| JP | 64-17066  | 1/1989  |
| JP | 1-299874  | 12/1989 |
| JP | 2-8256    | 1/1990  |
| JP | 3-101737  | 4/1991  |
| JP | 3-141363  | 6/1991  |
| JP | 3-191361  | 8/1991  |
| JP | 3-255456  | 11/1991 |
| JP | 3-269064  | 11/1991 |
| JP | 4-170552  | 6/1992  |
| JP | 5-80572   | 4/1993  |
| JP | 5-100461  | 4/1993  |

|    |            |         |
|----|------------|---------|
| JP | 5-210260   | 8/1993  |
| JP | 6-19174    | 1/1994  |
| JP | 6-208238   | 7/1994  |
| JP | 6-293769   | 10/1994 |
| JP | 7-271072   | 10/1995 |
| JP | 8-110649   | 4/1996  |
| JP | 11-5919    | 1/1999  |
| JP | 2001-19871 | 1/2001  |

## OTHER PUBLICATIONS

|                                                               |
|---------------------------------------------------------------|
| U.S. Appl. No. 11/219,886, filed Sep. 7, 2005, Niimi et al.   |
| U.S. Appl. No. 11/304,711, filed Dec. 16, 2005, Kondo et al.  |
| U.S. Appl. No. 11/332,545, Jan. 17, 2006, Tamoto et al.       |
| U.S. Appl. No. 11/367,786, Mar. 6, 2006, Ohta et al.          |
| U.S. Appl. No. 11/364,325, Mar. 1, 2006, Niimi.               |
| U.S. Appl. No. 11/474,258, Jun. 26, 2006, Niimi.              |
| U.S. Appl. No. 11/611,179, Dec. 15, 2006, Niimi et al.        |
| U.S. Appl. No. 11/749,292, May 16, 2007, Inaba et al.         |
| U.S. Appl. No. 11/625,873, filed Jan. 23, 2007, Niimi.        |
| U.S. Appl. No. 11/850,394, filed Sep. 5, 2007, Toshine et al. |
| U.S. Appl. No. 11/852,708, filed Sep. 10, 2007, Tada et al.   |
| U.S. Appl. No. 11/855,553, filed Sep. 14, 2007, Inaba et al.  |

\* cited by examiner

**FIG. 1**  
BAKGROUND ART



**FIG. 2**  
BAKGROUND ART



FIG. 3



FIG. 4



FIG. 5



FIG. 6



FIG. 7



FIG. 8



FIG. 9



FIG. 10



## FIG. 11



FIG. 12



FIG. 13



FIG.14



FIG. 15



FIG. 16



FIG. 17



FIG. 18



FIG. 19



FIG. 20



FIG. 21



**ELECTROPHOTOGRAPHIC  
PHOTORECEPTOR, METHOD FOR  
MANUFACTURING THE  
ELECTROPHOTOGRAPHIC  
PHOTORECEPTOR, AND IMAGE FORMING  
APPARATUS AND PROCESS CARTRIDGE  
USING THE ELECTROPHOTOGRAPHIC  
PHOTORECEPTOR**

**BACKGROUND OF THE INVENTION**

**1. Field of the Invention**

The present invention relates to an electrophotographic photoreceptor. Particularly the present invention relates to an electrophotographic photoreceptor having a photosensitive layer including a titanyl phthalocyanine crystal. In addition, the present invention also relates to a method for manufacturing the photoreceptor, and an image forming apparatus and a process cartridge using the electrophotographic photoreceptor.

**2. Discussion of the Background**

Recently, development of information processing systems utilizing electrophotography is remarkable. In particular, optical printers in which information is converted to digital signals and then the information is recorded using light have been dramatically improved in print qualities and reliability. This digital recording technique is applied to not only printers but also copiers, and so-called digital copiers have been developed. Copiers utilizing both the conventional analogue recording technique and this digital recording technique have various information processing functions, and therefore it is expected that demand for such copiers will be escalating. In addition, with popularization and improvement of personal computers, the performance of digital color printers which can produce documents including color images has been rapidly improved and broadly used.

Such digital image forming apparatus are required to be improved in functions year by year. Specifically digital image forming apparatus are required not only to have high durability and high stability but also to produce high quality images. On the other hand, in order to produce color images at a high speed, tandem image forming apparatus which include a plurality of image forming units each including image forming devices such as a photoreceptor, a charger, an image irradiator, an image developer, a cleaner and a quencher have been mainly used as the color image forming apparatus. In tandem image forming apparatus, yellow, magenta, cyan and black image forming units are provided side by side, and four color images concurrently formed in the respective image forming units are overlaid on an intermediate transfer medium or a receiving sheet. Thus, a color image can be formed at a high speed. In such tandem image forming apparatus, the image forming devices are required to be small in size to avoid jumboization of the image forming apparatus. In particular, it is essential that the photoreceptor used therefor have a small diameter. However, a photoreceptor which has a smaller diameter but has a shorter life cannot be used, and it is a problem to be solved how to develop a photoreceptor having a small diameter and a long life.

The life of a photoreceptor mainly depends on two factors, i.e., electrostatic fatigue thereof and the abrasion of the surface layer thereof. These are problems to be solved of the organic photoreceptors, which are mainly used now for the electrophotographic image forming apparatus. The former problem (electrostatic fatigue) is that when a photoreceptor is repeatedly subjected to image forming operations

such as charging and light irradiating, the electric potentials (potentials of lighted portions and non-lighted portions) formed on the photoreceptor change. In the case of organic photoreceptors, the potential of non-lighted portions typically decreases while the potential of lighted portions (i.e., residual potential) increases after repeated use. The latter problem is that the uppermost layer of a photoreceptor is mechanically abraded after repeated use by members contacting the photoreceptor such as cleaners. If the uppermost layer is thinned due to the abrasion, the strength of electric field formed on the photosensitive layer increases, resulting in acceleration of the electrostatic fatigue, and thereby the life of the photoreceptor is further shortened. In addition, when the surface of the photoreceptor is scratched by the contacting members, undesired images (such as streak images) are formed, resulting in shortening of the life of the photoreceptor. Therefore, these problems have to be solved at the same time, to develop a photoreceptor having a long life.

Recently, electrophotographic image forming apparatus can produce images at a high speed. Therefore, the image forming apparatus have also been used in printing fields. In order that electrophotographic image forming apparatus are used in printing fields, color images with high resolution higher than 600 dpi (dots per inch) have to be stably produced. In addition, the electrophotographic image forming apparatus have the following advantages over printing machines:

- (1) an original image can be directly reproduced at a high speed without making a plate; and
- (2) a large number of copies of an original image can be reproduced while a different information image is added to a part of each copy.

Therefore, the image forming apparatus (systems) are required to have good stability, namely the apparatus is required to stably produce high quality images without producing abnormal images.

Thus, long life and good stability are the important requisites for electrophotographic image forming apparatus. Among the image forming devices included in the electrophotographic image forming apparatus, the photoreceptor is the key device. As a result of studies of the electrostatic properties of photoreceptors and abrasion of the surface of photoreceptors, several technologies have been established.

For example, with respective to improvement in electrostatic properties, technologies such that (1) charge generation materials having a high photo-carrier generating efficiency are developed; and (2) charge transport materials having large mobility are developed have been established. By using a combination of such a charge generation material and a charge transport material, a photoreceptor having large gain and response in photo-decaying process can be provided. Therefore, by using such a photoreceptor for an image forming apparatus, the image forming apparatus can have the following advantages:

- (1) the potential (i.e., non-lighted potential) of the charged photoreceptor can be decreased;
- (2) the quantity of light used for optical writing can be decreased;
- (3) the developing bias can be decreased;
- (4) the transfer bias can be decreased; and
- (5) the quenching process can be eliminated.

Thus, the designing flexibility of the image forming apparatus can be increased. When these factors are minimized, the hazards for the photoreceptor can be eliminated, and thereby the designing flexibility of the photoreceptor can also be increased.

The usage of the photoreceptors used for high speed digital full color image forming apparatus is greatly different from that for analog image forming apparatus and monochrome image forming apparatus. For example, various optical writing methods are used in the full color image forming apparatus. In such full color image forming apparatus, production of abnormal images is typically caused by the photoreceptor used. Causes of abnormal images are broadly classified into the following two types. First, abnormal images are caused by scratches formed on the surface of the photoreceptor. Secondly, abnormal images are formed when the photoreceptor has electrostatic fatigue. In the first case, the production of abnormal images can be prevented to a considerable extent by improving the surface of the photoreceptor (for example, forming a protective layer as an uppermost layer) or improving the contacting members such as cleaners. In the second case, abnormal images (typically, background development) are caused by deterioration of the photoreceptor itself. Among the abnormal images, background development of images produced by a reverse (nega-posi) development method is a big problem now.

Specific examples of the cause for background development are as follows:

- (1) soils and defects of the electroconductive substrate used;
- (2) dielectric breakdown of the photosensitive layer;
- (3) injection of carriers (charges) from the substrate;
- (4) increase of dark decay of the photoreceptor; and
- (5) carriers thermally generated by a photoreceptor without irradiation of light to the photoreceptor (hereinafter referred to as hot carriers).

Among these causes, the soils and defects of the electroconductive substrate used can be removed before forming the photosensitive layer thereon, and therefore it is not avoidable. Therefore, in order to prevent occurrence of background development, it is considered to be important to improve the electric strength of the photoreceptor, to prevent carrier injection from the substrate and to decrease electrostatic fatigue of the photoreceptor.

From this point of view, techniques such that an undercoat layer or an intermediate layer is formed between the electroconductive substrate and the photoreceptor have been proposed. For example, published unexamined Japanese patent application No. (hereinafter referred to as JP-A) 47-6341 discloses an intermediate layer including a nitrocellulose, and JP-A 60-66258 discloses an intermediate layer including a nylon resin. In addition, JP-A 52-10138 discloses an intermediate layer including a maleic acid based resin, and JP-A 58-105155 discloses an intermediate layer including a polyvinyl alcohol resin.

However, these intermediate layers are a resin layer and have a high electric resistance. Therefore, the residual potential of the photoreceptor increases, resulting in decrease of image density when images are formed by a nega-posi developing method. In addition, such intermediate layers exhibit ionic conduction caused by impurities included therein, and therefore the electric resistance thereof increases particularly under low temperature and low humidity conditions, resulting in increase of the residual potential. Therefore, the intermediate layer has to be thinned, and thereby a problem in that the charge properties and charge retainability of the photoreceptor deteriorate after repeated use occurs.

In attempting to solve this problem (i.e., in attempting to control the resistance of an intermediate layer), techniques in that an electroconductive material is included in an intermediate layer have been proposed. For example, JP-A 51-65942 discloses an intermediate layer in which carbon or

chalogen materials is dispersed in a crosslinked resin. JP-A 52-82238 discloses an intermediate layer which is crosslinked using an isocyanate crosslinking agent upon application of heat thereto and which includes a quaternary ammonium salt. JP-A 55-113045 discloses a resinous intermediate layer including a resistance controlling agent. JP-A 58-93062 discloses a resinous intermediate layer including an organic metal compound. However, the photoreceptors including such resinous intermediate layers have a drawback in that images having moiré fringes are produced when the photoreceptors are used for image forming apparatus using coherent light such as laser light for image writing.

In attempting to solve the resistance and moiré fringe problems, intermediate layers including a filler have been proposed. For example, JP-A 58-58556 discloses a resinous intermediate layer including aluminum oxide or tin oxide. JP-A 60-111255 discloses a resinous intermediate layer including a particulate electroconductive material. JP-A 59-17557 discloses an intermediate layer including magnetite. JP-A 60-32054 discloses a resinous intermediate layer including titanium oxide and tin oxide. JP-As 64-68762, 64-68763, 64-73352, 64-73353, 01-118848 and 01-118849 have disclosed resinous intermediate layers including a powder such as borides, nitrides, fluorides and oxides. In these resinous intermediate layers including a filler, the content of the filler in the intermediate layer has to be increased (i.e., the content of the resin has to be decreased) so that the intermediate layer has the desired electric properties. Therefore, the adhesion of the intermediate layer to the electroconductive substrate deteriorates, and thereby a problem in that the intermediate layer is separated from the electroconductive substrate tends to occur. Particularly, when the substrate is a flexible belt, the problem occurs more frequently.

In attempting to solve the problem, techniques in that a layered intermediate layer is provided have been proposed. The layered intermediate layers are broadly classified into two types, which have structures as illustrated in FIGS. 1 and 2. The first type of the intermediate layers, which is illustrated in FIG. 1, includes an electroconductive substrate 1, a resin layer 2 including a filler, a resin layer 3 including no filler, and a photosensitive layer 4, which are overlaid in this order. The second type of the intermediate layers, which is illustrated in FIG. 2, includes an electroconductive substrate 1, a resin layer 3 including no filler, a resin layer 2 including a filler and a photosensitive layer 4 which are overlaid in this order.

Specifically, in the first type intermediate layer, the electroconductive layer 2 which includes a filler having a low electric resistance is formed on the electroconductive substrate 1. In addition, the resin layer 3 is formed thereon. The intermediate layers of this type have been disclosed in JP-As 58-95351, 59-93453, 04-170552, 06-208238, 06-222600, 08-184979, 09-43886, 09-190005 and 09-288367.

In the intermediate layers of this type, the electroconductive layer 2 serves as an electrode. Therefore the intermediate layer is electrically the same as the resinous intermediate layer, and thereby the above-mentioned electrostatic problem of the photoreceptor having a resinous intermediate layer cannot be solved. Since the electroconductive layer includes a filler, occurrence of moiré fringes can be prevented because the light beam for image writing scatter. When such a photoreceptor is charged, charges having a polarity opposite to that of the charges formed on the surface of the photoreceptor reach the interface between the electroconductive layer 2 and the resinous layer 3. However, when the electroconductive layer 2 has a relatively high

resistance, charges are not well injected from the electroconductive substrate 1, and the resistance of the layer 2 increases after long repeated use, thereby increasing the residual potential of the photoreceptor. In addition, in order to avoid the problem caused by defects of the electroconductive substrate 1, the layer 2 has to have a thickness not less than about 10  $\mu\text{m}$ . In this case, the residual potential increasing problem remarkably occurs.

JP-As 05-100461, 05-210260 and 07-271072 have disclosed photoreceptors in which an electroconductive layer, an intermediate layer and a photosensitive layer including a titanylphthalocyanine crystal, which are overlaid in this order. However, the crystal form and the primary particle diameter of the titanyl phthalocyanine crystal are not controlled. Therefore, occurrence of the background development problem due to the hot carriers cannot be prevented.

In the second type intermediate layer, a positive hole blocking layer is formed on the electroconductive substrate, and a resin layer including a filler having a low resistance or an electroconductive filler is formed on the positive hole blocking layer. These intermediate layers have been disclosed in JP-As 05-80572 and 06-19174. The photoreceptors of this type hardly cause the background development problem because the intermediate layer has a positive hole blocking function. In addition, since a filler-including layer is present thereon, residual potential hardly increases. Specifically, injection of positive holes from the electroconductive substrate 1 to the photosensitive layer 4 can be avoided, and thereby the background development problem in a nega-posi development method hardly occurs. In addition, since a charge blocking layer is formed as a lower layer, the degree of increase of residual potential of the photoreceptor after long repeated use is lower than in the case where the charge blocking layer is formed as an upper layer.

However, the background development is caused by not only charges injected from the electroconductive substrate to the photosensitive layer but also carriers thermally generated in the photosensitive layer. If a proper charge generation material is not used for the charge generation layer and the conditions of the particles of the charge generation material are not properly controlled, occurrence of the background development problem cannot be prevented.

Because of these reasons, a need exists for an electrophotographic photoreceptor which can stably produce images without causing the problems mentioned above.

#### SUMMARY OF THE INVENTION

Accordingly, an object of the present invention is to provide a photoreceptor which can stably produce images for a long period of time without causing problems such as the background development problem (i.e., increase of residual potential), and the dielectric breakdown problem.

Another object of the present invention is to provide an image forming apparatus and a process cartridge which can produce high quality images for a long period of time without causing the problems mentioned above and without frequently changing the photoreceptor.

Briefly these objects and other objects of the present invention as hereinafter will become more readily apparent can be attained by a photoreceptor including at least an electroconductive substrate, and a charge blocking layer, a moiré preventing layer, and a photosensitive layer, which are located overlying the electroconductive substrate in this order, wherein the photosensitive layer includes a titanyl phthalocyanine crystal which has an average primary particle diameter not greater than 0.25  $\mu\text{m}$  and has a first X-ray

diffraction spectrum such that a maximum peak is observed at a Bragg (20) angle of  $27.2^\circ \pm 0.2^\circ$ ; a peak is observed at Bragg (20) angle of  $9.4^\circ \pm 0.2^\circ$ ,  $9.6 \pm 0.2^\circ$  and  $24.0 \pm 0.2^\circ$ ; a lowest angle peak is observed at an angle of  $7.3^\circ \pm 0.2^\circ$ ; no peak is observed between the lowest angle peak and the  $9.4^\circ$  peak; and no peak is observed at a Bragg (20) angle of  $26.3^\circ \pm 0.2^\circ$ , when a Cu—K $\alpha$  X-ray having a wavelength of 1.542  $\text{\AA}$  is used.

In this regard, "overlying" can include direct contact and allow for intermediate layers.

The photosensitive layer preferably includes a charge generation layer including the titanyl phthalocyanine crystal and a charge transport layer which are overlaid.

The photosensitive layer or the charge generation layer is preferably prepared using a coating liquid prepared by a method including the steps of dispersing the titanyl phthalocyanine crystal in a solvent such that the titanyl phthalocyanine crystal therein has a particle diameter distribution such that an average particle diameter is not greater than 0.3  $\mu\text{m}$  and a standard deviation is not greater than 0.2  $\mu\text{m}$  to prepare a dispersion; and filtering the dispersion using a filter having an effective pore diameter not greater than 3  $\mu\text{m}$ .

The titanyl phthalocyanine crystal is preferably prepared by a method including the steps of providing a titanyl phthalocyanine pigment (raw material) having an amorphous state or a low crystallinity (hereinafter referred to as phthalocyanine pigment having an amorphous state or amorphous titanyl phthalocyanine), which has an average particle diameter not greater than 0.1  $\mu\text{m}$  and has a second X-ray diffraction spectrum such that a maximum peak having a half width not less than  $1^\circ$  is observed at a Bragg (20) angle of from  $7.0^\circ$  to  $7.5^\circ$  with a tolerance of  $\pm 0.2^\circ$ ; changing the crystal form of the amorphous titanyl phthalocyanine in an organic solvent in the presence of water so that the resultant titanyl phthalocyanine crystal has the above-mentioned X-ray diffraction spectrum; and filtering the dispersion including the titanyl phthalocyanine crystal before the average primary particle diameter thereof exceeds 0.25  $\mu\text{m}$ , to prepare the titanyl phthalocyanine crystal.

The titanyl phthalocyanine crystal is preferably synthesized using raw materials including no halogen atom.

The amorphous titanyl phthalocyanine is preferably prepared by an acid paste method, and then washed using ion-exchanged water to an extent such that the ion-exchange water used for washing have a pH of from 6 to 8 and/or a specific conductivity not greater than 8.

In the crystal changing process, the amount of the organic solvent is preferably not less than 30 times that of the amorphous titanyl phthalocyanine.

It is preferable that the charge blocking layer includes an insulating material, which is preferably a polyamide, and has a thickness less than 2.0  $\mu\text{m}$ .

It is preferable that the moiré preventing layer includes an inorganic pigment and a binder resin, wherein the volume ratio (P/R) of the inorganic pigment (P) to the binder resin (R) is from 1/1 to 3/1. The binder resin is preferably a thermosetting resin, which is preferably a mixture of an alkyd resin and a melamine resin. The weight ratio (A/M) of the alkyd resin (A) to the melamine resin (M) is preferably from 5/5 to 8/2. The inorganic pigment is preferably titanium oxide. The titanium oxide is preferably a mixture of a titanium oxide (T1) having an average particle diameter of D1, and another titanium oxide (T2) having an average particle diameter of D2, wherein the relationship  $0.2 < (D2/D1) \leq 0.5$  is satisfied. The average particle diameter D2 is greater than 0.05  $\mu\text{m}$  and less than 0.2  $\mu\text{m}$ . The titanium

oxides T1 and T2 are preferably mixed in such a weight ratio that the following relationship is satisfied:

$$0.2 \leq T2/(T1+T2) \leq 0.8.$$

It is preferable that the photoreceptor further includes a protective layer located overlying the photosensitive layer. The protective layer preferably includes an inorganic pigment such as metal oxides having a resistivity not less than  $10^{10}$   $\Omega\text{-cm}$ . The inorganic pigment is preferably selected from the group consisting of alumina, titanium oxide and silica. More preferably, the inorganic pigment is  $\alpha$ -alumina. The protective layer preferably includes a charge transport polymer. The protective layer preferably includes a crosslinked binder resin, which preferably includes a charge transport moiety therein.

As another aspect of the present invention, a method for manufacturing the photoreceptor is provided which includes the steps of:

- forming the charge blocking layer overlying the electro-conductive substrate;
  - forming the moiré preventing layer overlying the charge blocking layer;
  - forming the charge generation layer overlying the moiré preventing layer; and
  - forming the charge transport layer overlying the charge generation layer,
- wherein the charge generation layer forming step includes:
- providing an amorphous titanyl phthalocyanine which has an average particle diameter not greater than 0.1  $\mu\text{m}$  and has a second X-ray diffraction spectrum such that a maximum peak having a half width not less than  $1^\circ$  is observed at a Bragg (20) angle of from  $7.0^\circ$  to  $7.5^\circ$  with a tolerance of  $\pm 0.2^\circ$ ;
  - changing a crystal form of the amorphous titanyl phthalocyanine in an organic solvent in the presence of water so that the titanyl phthalocyanine has the first X-ray diffraction spectrum; and filtering the dispersion including the crystal-changed titanyl phthalocyanine before the average primary particle diameter exceeds 0.25  $\mu\text{m}$ , to prepare the titanyl phthalocyanine crystal;
  - preparing a coating liquid which includes at least the titanyl phthalocyanine crystal and a solvent and in which the titanyl phthalocyanine crystal is dispersed in the solvent while having a particle diameter distribution such that an average particle diameter is not greater than 0.3  $\mu\text{m}$  and a standard deviation is not greater than 0.2  $\mu\text{m}$ ;
  - filtering the coating liquid using a filter having an effective pore diameter not greater than 3  $\mu\text{m}$ ;
  - coating the coating liquid overlying the moiré preventing layer; and
  - drying the coated liquid.

As another aspect of the present invention, an image forming apparatus is provided which includes the photoreceptor mentioned above, a charger configured to charge the photoreceptor, a light irradiator configured to irradiate the photoreceptor with imagewise light to form an electrostatic latent image, a developing device configured to develop the electrostatic latent image with a developer including a toner to form a toner image on the photoreceptor, and a transfer device configured to transfer the toner image onto a receiving material optionally via an intermediate transfer medium. The image forming apparatus can include a plurality of

image forming units each including the photoreceptor, charger, light irradiator, developing device and transfer device.

The charger is preferably a contact charger or a short-range charger which charges the photoreceptor while a small gap (preferably not greater than 100  $\mu\text{m}$ ) is formed between the surface of the charger and the surface of the photoreceptor. The charger preferably applies a DC voltage overlapped with an AC voltage.

10 The image forming apparatus preferably includes a process cartridge which includes the photoreceptor mentioned above and at least a device selected from the group consisting of chargers, light irradiators, developing devices and cleaning devices and which can be detachably set in the image forming apparatus.

15 As a further aspect of the present invention, a process cartridge is provided which includes the photoreceptor mentioned above and at least a device selected from the group consisting of a charger, a light irradiator, a developing device and a cleaner.

20 These and other objects, features and advantages of the present invention will become apparent upon consideration of the following description of the preferred embodiments of the present invention taken in conjunction with the accompanying drawings.

#### BRIEF DESCRIPTION OF THE DRAWINGS

30 Various other objects, features and attendant advantages of the present invention will be more fully appreciated as the same becomes better understood from the detailed description when considered in connection with the accompanying drawings in which like reference characters designate like corresponding parts throughout and wherein:

35 FIG. 1 is a schematic cross sectional view for explaining a conventional photoreceptor;

FIG. 2 is a schematic cross sectional view for explaining another conventional photoreceptor;

40 FIG. 3 is a photograph showing a titanyl phthalocyanine raw material having an amorphous state, which is taken using a transmission electron microscope;

FIG. 4 is a photograph showing primary particles of a titanyl phthalocyanine crystal prepared by subjecting the titanyl phthalocyanine raw material to a crystal changing treatment, which is taken using a transmission electron microscope;

FIG. 5 is a photograph showing primary particles of a titanyl phthalocyanine crystal prepared by rapidly performing the crystal changing treatment, which is taken using a transmission electron microscope;

FIGS. 6 and 7 are photographs showing the dispersion states of the titanyl phthalocyanine crystal in different dispersions A and B which are prepared by the same method except that the dispersion time is changed;

55 FIG. 8 is a graph showing the particle diameter distributions of the dispersions A and B;

FIGS. 9-11 are schematic cross sectional views illustrating examples of the photoreceptor of the present invention;

60 FIG. 12 is a schematic view illustrating an embodiment of the image forming apparatus of the present invention;

FIG. 13 is a schematic view illustrating an embodiment of the short-range charger for use in the image forming apparatus of the present invention;

65 FIG. 14 is a schematic view illustrating another embodiment of the image forming apparatus of the present invention;

FIG. 15 is a schematic view illustrating an embodiment of the process cartridge of the present invention;

FIG. 16 is a schematic view illustrating another embodiment (tandem full color image forming apparatus) of the image forming apparatus of the present invention;

FIG. 17 is the X-ray diffraction spectrum of the titanyl phthalocyanine crystal prepared in Comparative Synthesis Example 1;

FIG. 18 is the X-ray diffraction spectrum of the titanyl phthalocyanine pigment obtained by drying the wet paste prepared in Comparative Synthesis Example 1;

FIG. 19 is the X-ray diffraction spectrum of the titanyl phthalocyanine crystal prepared in Comparative Synthesis Example 9;

FIG. 20 is the X-ray diffraction spectrum of the pigment prepared in Measurement Example 1; and

FIG. 21 is the X-ray diffraction spectrum of the pigment prepared in Measurement Example 2.

#### DETAILED DESCRIPTION OF THE INVENTION

At first, the photoreceptor of the present invention will be explained in detail.

The photoreceptor of the present invention including at least an electroconductive substrate, and a charge blocking layer, a moiré preventing layer, and a photosensitive layer, which are located overlying the electroconductive substrate in this order, wherein the photosensitive layer includes a titanyl phthalocyanine crystal which has an average primary particle diameter not greater than 0.25  $\mu\text{m}$  and has an X-ray diffraction spectrum such that a maximum peak is observed at a Bragg (20) angle of  $27.2^\circ \pm 0.2^\circ$ ; a peak is observed at Bragg (20) angle of  $9.4^\circ \pm 0.2^\circ$ ,  $9.6^\circ \pm 0.2^\circ$  and  $24.0^\circ \pm 0.2^\circ$ ; a lowest angle peak is observed at an angle of  $7.3^\circ \pm 0.2^\circ$ ; no peak is observed between the lowest angle peak and the  $9.4^\circ$  peak; and no peak is observed at a Bragg (20) angle of  $26.3^\circ \pm 0.2^\circ$ , when a Cu—K $\alpha$  X-ray having a wavelength of 1.542  $\text{\AA}$  is used.

The crystal form of titanyl phthalocyanine is described in JP-A 2001-19871. By using such a titanyl phthalocyanine crystal for a photosensitive layer, the resultant photoreceptor has high sensitivity and can maintain good charge properties even after long repeated use. JP-A 2001-19871 discloses the charge generation material (i.e., the titanyl phthalocyanine crystal having the same crystal form), a photoreceptor including the titanyl phthalocyanine crystal and an image forming apparatus using the photoreceptor. However, when such a photoreceptor is repeatedly used for forming images with a resolution not less than 600 dpi or 1200 dpi for a long period of time, the photoreceptor causes the background development problem, namely the photoreceptor does not have a long life. This background development problem is caused particularly when the photoreceptor is used for image forming apparatus which produce images at a speed higher than that of the image forming apparatus described in JP-A 2001-19871.

As a result of the present inventors' investigation, it is found that the problem can be solved by controlling the particle size of the titanyl phthalocyanine crystal. Thus, in the photoreceptor of the present invention, the ability of the titanyl phthalocyanine crystal can be fully exhibited.

On the other hand, the technique such that an intermediate layer in which a charge blocking layer and a moiré preventing layer are overlaid is formed between an electroconductive substrate and a photosensitive layer is described in, for example, JP-A 05-80572. However, when such an interme-

diate layer is used in combination with a photosensitive layer having a high sensitivity, the background development problem is not perfectly avoided because the charge property of the photosensitive layer is affected by the hot carriers. 5 This problem is more frequently caused when such a charge generation material as to have absorption in a relatively long wavelength like the titanyl phthalocyanine mentioned above for use in the present invention is used.

Thus, the techniques are partially completed. Specifically, 10 the photoreceptors having a charge blocking layer, a moiré preventing layer and a photosensitive layer including the titanyl phthalocyanine crystal having the specific crystal form have high photosensitivity and good charge stability, but cannot well solve the problems such as background development and dielectric breakdown.

As a result of the present inventors' investigation, it is found that by combining the techniques with a technique in that the particle diameter of the titanyl phthalocyanine crystal is controlled so as to be not greater than 0.25  $\mu\text{m}$ , the 20 objects of the present invention can be attained.

Then the method for synthesizing the titanyl phthalocyanine crystal having the specific crystal form mentioned above will be explained.

At first, the method for synthesizing crude titanyl phthalocyanine will be explained. The method for synthesizing titanyl phthalocyanine is well known and several methods have been described in "Phthalocyanine Compounds" (1963) and "The Phthalocyanines" (1983) by Moser, and JP-A 06-293769.

For example, one method is that a mixture of maleic anhydrides, a metal or a halogenated metal, and urea is heated in the presence or absence of a solvent having a high boiling point. In this case, a catalyst such as ammonium molybdate is used if desired. The second method is that a mixture of phthalonitriles and a halogenated metal is heated in the presence of absence of a solvent having a high boiling point. This method is used for synthesizing phthalocyanines such as aluminum phthalocyanines, indium phthalocyanines, oxovanadium phthalocyanines, oxotitanium phthalocyanines, zirconium phthalocyanines, etc., which cannot be synthesized by the first method. The third method is that maleic anhydride or one of phthalonitriles is reacted with ammonia to produce an intermediate such as 1,3-diminoisoindoline, followed by reaction of the intermediate with a halogenated metal in a solvent having a high boiling point. The fourth method is that one of phthalonitriles is reacted with a metal alkoxide in the presence of urea, etc. Since the fourth method has an advantage in that the benzene ring is not halogenated, the method is preferably used for synthesizing the titanyl phthalocyanine crystal for use in electro-photography. Therefore, the method is preferably used in the present invention.

Thus, the titanyl phthalocyanine crystal for use in the present invention is preferably synthesized by a method 55 which is described in JP-A 06-293769 and which does not use a halogenated titanium. The greatest advantage of this method is that the synthesized titanyl phthalocyanine is free from halogen. When a titanyl phthalocyanine crystal which includes a halogenated titanyl phthalocyanine crystal as an 60 impurity is used for a photoreceptor, the photoreceptor has low photosensitivity and poor charge properties as described in Japan Hardcopy '89 p. 103, 1989. The halogen-free titanyl phthalocyanine is preferably used for the photoreceptor of the present invention.

65 Then the method for synthesizing the amorphous titanyl phthalocyanine will be explained. In this case, acid paste methods or acid slurry methods in which a crude phthalo-

## 11

cyanines is dissolved in sulfuric acid and the solution is diluted with water to re-precipitate the phthalocyanine are preferably used.

Specifically, the procedure is as follows:

- (1) the crude titanyl phthalocyanine prepared above is dissolved in concentrated sulfuric acid having a weight of from 10 to 50 times that of the crude titanyl phthalocyanine;
- (2) materials remaining undissolved in sulfuric acid are removed therefrom by filtering, etc.;
- (3) the solution is added to an ice water having a weight of from 10 to 50 times that of the sulfuric acid used, to precipitate an amorphous titanyl phthalocyanine;
- (4) after the amorphous titanyl phthalocyanine is separated by filtering, the titanyl phthalocyanine is repeatedly subjected to washing with ion-exchange water and filtering until the filtrate becomes neutral; and
- (5) the amorphous titanyl phthalocyanine is washed with ion-exchange water, followed by filtering to prepare an aqueous paste having a solid content of from 5 to 15% by weight.

In this case, it is important to well wash the amorphous titanyl phthalocyanine so that the amount of sulfuric acid in the aqueous paste becomes as small as possible. Specifically, the filtrate (i.e., water used for washing the titanyl phthalocyanine) preferably has a pH of from 6 to 8 and/or a specific conductivity not greater than 8. It is found that when the pH and/or the specific conductivity of the filtrate fall in the range mentioned above, the properties of the resultant photoreceptor are not affected by the sulfuric acid remaining in the titanyl phthalocyanine crystal. The pH and specific conductivity can be measured with a marketed pH meter and a marketed electric conductivity measuring instrument, respectively. The lower limit of the specific conductivity of the filtrate is the specific conductivity of the ion-exchange water used for washing.

When the pH and specific conductivity do not fall in the above-mentioned ranges (i.e., the amount of residual sulfuric acid is large), the resultant photoreceptor has low photosensitivity and poor charge properties.

Thus, the amorphous titanyl phthalocyanine (raw material) can be prepared. The amorphous titanyl phthalocyanine preferably has an X-ray diffraction spectrum such that a maximum peak is observed at a Bragg (20) angle of from 7.0° to 7.5° with a tolerance of  $\pm 0.2^\circ$  when a Cu—K $\alpha$  X-ray having a wavelength of 1.542 Å is used. In addition, the half width of the maximum peak is preferably not less than 1°. Further, the average particle diameter of the primary particles thereof is preferably not greater than 0.1  $\mu\text{m}$ .

Then the method for changing the crystal form will be explained.

In the crystal form changing process, the amorphous titanyl phthalocyanine is changed to a titanyl phthalocyanine crystal which has an X-ray diffraction spectrum such that a maximum peak is observed at a Bragg (20) angle of  $27.2^\circ \pm 0.2^\circ$ ; a peak is observed at Bragg (20) angle of  $9.4^\circ \pm 0.2^\circ$ ,  $9.6^\circ \pm 0.2^\circ$  and  $24.0^\circ \pm 0.2^\circ$ ; a lowest angle peak is observed at an angle of  $7.3^\circ \pm 0.2^\circ$ ; no peak is observed between the lowest angle peak and the  $9.4^\circ$  peak; and no peak is observed at a Bragg (20) angle of  $26.3^\circ \pm 0.2^\circ$ , when a Cu—K $\alpha$  X-ray having a wavelength of 1.542 Å is used.

Specifically, the desired titanyl phthalocyanine crystal can be prepared by mixing the amorphous above-prepared titanyl phthalocyanine, which is not dried, with an organic solvent in the presence of water while agitating.

Suitable solvents for use in the crystal form changing process include any known solvents by which the desired

## 12

titanyl phthalocyanine crystal can be prepared. In particular, it is preferable to use one or more of tetrahydrofuran, toluene, methylene chloride, carbon disulfide, and o-dichlorobenzene, 1,1,2-trichloroethane. It is preferable to use one of these solvents alone. However, mixtures thereof can also be used. In addition, other solvents can be added to the solvents.

The amount of the solvent used for the crystal form changing process is preferably not less than 10 times, 10 more preferably not less than 30 times, the weight of the titanyl phthalocyanine used. This is because the crystal change can be rapidly performed and in addition the impurities included in the titanyl phthalocyanine can be well removed. As mentioned above, the amorphous titanyl phthalocyanine used for the crystal changing process is typically prepared by an acid paste method. In this case, it is preferable to fully wash the amorphous titanyl phthalocyanine to remove sulfuric acid therefrom. When sulfuric acid is not fully removed from the amorphous titanyl phthalocyanine, sulfate ions are included in the resultant titanyl phthalocyanine crystal even after the crystal is well washed. When sulfate ions are included in the crystal, the resultant photoreceptor has a low photosensitivity and poor charge properties.

For example, JP-A 08-110649 discloses a crystal changing method in a comparative example therein, in which a titanyl phthalocyanine which is dissolved in sulfuric acid and water are added to an organic solvent to change the crystal form of the titanyl phthalocyanine. The resultant titanyl phthalocyanine crystal has an X-ray diffraction spectrum similar to that of the titanyl phthalocyanine crystal of the present invention. However, the titanyl phthalocyanine crystal includes sulfate ions at a high concentration. Therefore, the resultant photoreceptor has low photosensitivity. 35 Namely, the method is not preferable and cannot be used for preparing the titanyl phthalocyanine crystal for use in the present invention.

The thus prepared titanyl phthalocyanine crystal preferably has a small particle diameter to increase the effect 40 thereof. The methods for preparing such a titanyl phthalocyanine crystal will be explained.

The methods are broadly classified into two methods. One of the methods is that the titanyl phthalocyanine crystal is synthesized while controlling the particle diameter of the 45 crystal so as not greater than 0.25  $\mu\text{m}$ . The other method is that when the titanyl phthalocyanine crystal is dispersed, coarse particles having a particle diameter greater than 0.25  $\mu\text{m}$  are removed therefrom. Needless to say, it is more preferable to use both the methods.

At first, the method for synthesizing a titanyl phthalocyanine crystal having a small particle diameter will be explained.

As a result of the present inventors' investigation of 55 synthesizing a titanyl phthalocyanine crystal having a small particle diameter, the following knowledge can be acquired. Specifically, it is found that the titanyl phthalocyanine having an irregular form (low crystallinity) typically has a primary particle diameter not greater than 0.1  $\mu\text{m}$  (almost all the particles have a primary particle diameter of from 0.01 to 0.05  $\mu\text{m}$ ) as can be understood from FIG. 3. In FIG. 3, the practical length of the scale bar is 0.2  $\mu\text{m}$ . In addition, it is found that the crystal change is performed with crystal growth.

In general, in such a crystal changing process, the crystal 60 changing operation is performed for a relatively long time to fully perform the crystal changing, i.e., to prevent inclusion of the raw material in the product. Then the product is

filtered to prepare the titanyl phthalocyanine crystal having the desired crystal form. Therefore, even though the titanyl phthalocyanine raw material has a small particle diameter, the resultant titanyl phthalocyanine crystal typically has a relatively large particle diameter (from about 0.3 to about 0.5  $\mu\text{m}$ ) as can be understood from FIG. 4. In FIG. 4, the practical length of the scale bar is 0.2  $\mu\text{m}$ . The thus prepared titanyl phthalocyanine crystal is dispersed while applying a high shearing force thereto such that the particle diameter thereof becomes not greater than 0.25  $\mu\text{m}$ . In addition, the titanyl phthalocyanine crystal is pulverized if necessary. Therefore, a problem in that part of the crystal has a crystal form different from the desired crystal form occurs.

In contrast, in the present invention the crystal change is completed while the crystal growth hardly occurs. Specifically, the particle diameter of the resultant titanyl phthalocyanine crystal has almost the same particle diameter (not greater than about 0.2  $\mu\text{m}$ ) as that of the amorphous titanyl phthalocyanine (raw material). The particle diameter of the crystal increases in proportion to the time during which the crystal changing is performed. Therefore, it is important that the crystal changing efficiency is enhanced to complete the crystal changing operation in a short time, and the following is the key points.

Specifically, one of the key points is that the proper solvents as mentioned above are used for the crystal changing process. Another key point is that the aqueous paste of the amorphous titanyl phthalocyanine is efficiently contacted with the solvent in the crystal changing process by performing strong agitation. Specifically, the amorphous titanyl phthalocyanine is preferably mixed with the solvent using a dispersion machine which can perform strong agitation using a propeller, such as homogenizers (e.g., HOMO-MIXER). By using these methods, the crystal changing operations can be completed in a short time. Namely, a titanyl phthalocyanine crystal in which crystal change is fully performed (i.e., which hardly includes the raw material) without causing crystal growth can be prepared.

Even in this case, it is important to use a proper amount of solvent for crystal changing as mentioned above. Specifically, the amount of the solvent is preferably not less than 10 times, and more preferably not less than 30 times, the amount of the amorphous titanyl phthalocyanine (raw material) used. By using this method, the crystal changing can be completed in a short time while preventing the impurities included in the titanyl phthalocyanine raw material from remaining in the resultant titanyl phthalocyanine crystal.

As mentioned above, the particle diameter of the titanyl phthalocyanine crystal increases in proportion to the crystal changing time. Therefore, it is also effective to rapidly stop the crystal changing reaction when crystal changing is completed. In order to rapidly stop the reaction, it is preferable to add a large amount of second solvent, by which crystal changing is hardly caused, to the system. Specific examples of such second solvents include alcohol solvents and ester solvents. The ratio of the second solvent to the crystal changing solvent is preferably about 10/1.

With respect to the thus prepared titanyl phthalocyanine crystal, the smaller particle diameter the crystal has, the better properties the resultant photoreceptor has. However, when the particle diameter is too small, problems in that filtering takes a relatively long time and the dispersion stability of the dispersion including the crystal deteriorates (i.e., the primary particles aggregate because the surface area of the particles increases) tend to occur. Therefore, the particle diameter of the titanyl phthalocyanine crystal is preferably from 0.05  $\mu\text{m}$  to 0.2  $\mu\text{m}$ .

FIG. 5 is a photograph showing a titanyl phthalocyanine crystal which is prepared by performing crystal change in a short time. In FIG. 5, the practical length of the scale bar is 0.2  $\mu\text{m}$ . As can be understood from FIGS. 4 and 5, the crystal as shown in FIG. 5 has a small average particle diameter and variation of the particle diameter is small. In addition, the crystal as shown in FIG. 5 includes no coarse particles whereas the crystal as shown in FIG. 4 includes coarse particles.

The thus prepared titanyl phthalocyanine crystal can be dispersed even when such a high shearing force as applied for the crystals including coarse particles is not applied thereto. Therefore, a dispersion including a crystal having an average particle diameter not greater than 0.25  $\mu\text{m}$  (preferably not greater than 0.20  $\mu\text{m}$ ) can be easily prepared without causing a problem in that part of the crystal causes crystal change.

In the present application, the particle diameter means the volume average particle diameter, and can be determined by a centrifugal automatic particle diameter analyzer, CAPA-700 from Horiba Ltd. The volume average particle diameter means the cumulative 50% particle diameter (i.e., Median diameter). However, by using this method, there is a case where a small amount of coarse particles cannot be detected. Therefore, it is preferable to directly observe the dispersion including a titanyl phthalocyanine crystal with an electron microscope, to determine the particle diameter of the crystal.

In addition, with respect to minute coating defects in a layer formed using a titanyl phthalocyanine crystal dispersion, the following knowledge can be acquired. The presence of coarse particles in the dispersion can be detected by a particle diameter measuring instrument if the concentration of coarse particles is on the order of a few percent or more. However, when the concentration is not greater than 1%, the presence of coarse particles cannot be detected by such an instrument. Therefore, even when it is confirmed that the average particle diameter of the crystal in a dispersion falls in the preferable range, a problem in that the resultant charge generation layer has minute coating defects can occur.

FIGS. 6 and 7 are photographs showing the dispersion state of the titanyl phthalocyanine crystal in different dispersions A and B which are prepared by the same method except that the dispersion time is changed. The dispersion time for the dispersion A is shorter than that for the dispersion B. As can be understood from FIG. 6, coarse particles are present in the dispersion A. Coarse particles are observed as black spots in FIG. 6.

The particle diameter distributions of the dispersions A and B, which are measured with a centrifugal automatic particle diameter analyzer, CAPA-700 from Horiba Ltd., are illustrated in FIG. 8. In FIG. 8, characters A and B represent the particle diameter distributions of the dispersions A and B, respectively. As can be understood from the graph, the particle diameter distributions are almost the same. The average particle diameters of the dispersions A and B are 0.29 and 0.28  $\mu\text{m}$ , respectively, which are the same when considering the measurement error. Thus, whether or not coarse particles are present cannot be determined by such a method in which the average particle diameter is measured by such a particle diameter measuring instrument. As mentioned above, the presence of coarse particles can be detected only by the method in which a dispersion is directly observed using a microscope.

Under such circumstances, it is very effective that the primary particle diameter of the titanyl phthalocyanine crys-

## 15

tal is controlled so as to be as small as possible in the crystal changing process. Specifically, the following is the key points:

- (1) such a proper solvent as mentioned above is used as the solvent in the crystal changing process to increase the crystal change efficiency; and
- (2) an aqueous titanyl phthalocyanine paste (i.e., an aqueous paste of amorphous titanyl phthalocyanine) is well contacted with the solvent by performing strong agitation in the crystal changing process to rapidly complete crystal changing.

By using this method, a titanyl phthalocyanine crystal having a small primary particle diameter (i.e., not greater than 0.25  $\mu\text{m}$ , and preferably not greater than 0.2  $\mu\text{m}$ ) can be prepared. In addition, it is very effective for heighten the effects of the present invention to use this method in combination with the method described in 2001-19871 mentioned above.

The thus prepared titanyl phthalocyanine crystal is preferably filtered rapidly using a filter with a proper pore size to separate the crystal from the solvent. In this case, the filtration is preferably performed under a reduced pressure.

The thus prepared titanyl phthalocyanine crystal is heated to be dried, if necessary. Any known heating dryers can be used for drying the crystal, but fan heaters are preferably used when drying is performed under normal pressure. In order to increase the drying speed and to enhance the effects of the present invention, it is preferable to perform drying under a reduced pressure. Particularly, this method is useful for materials which decompose or cause crystal change at a high temperature. The pressure is preferably not higher than 10 mmHg when drying is performed under a reduced pressure.

The thus prepared titanyl phthalocyanine crystal having such a specific crystal form as mentioned above is preferably used as a charge generation material for use in electrophotographic photoreceptors. As mentioned above, by using conventional methods for preparing a dispersion, titanyl phthalocyanine crystal easily causes crystal change. However, by using the above-mentioned method of the present invention, a dispersion including the titanyl phthalocyanine crystal having a small particle diameter can be prepared without applying so high a shearing force thereto. Accordingly, the titanyl phthalocyanine crystal does not cause crystal change in the dispersing process.

Next, a method for removing coarse particles from a dispersion will be explained.

A dispersion including the titanyl phthalocyanine crystal is prepared by dispersing the crystal, optionally together with a binder resin, in a solvent using a ball mill, an attritor, a sand mill, a bead mill, an ultrasonic dispersing machine or the like. In this case, it is preferable that a proper resin is chosen in consideration of the electrostatic properties of the resultant photoreceptor and a proper solvent is chosen in consideration of its abilities to wet and disperse the crystal.

As mentioned above, it is known that the titanyl phthalocyanine crystal having an X-ray diffraction peak such that a maximum peak is present at Bragg (20) angle of  $27.2^\circ \pm 0.2^\circ$  easily causes crystal change when a stress (such as heat energy and mechanical shearing force) is applied thereto. The titanyl phthalocyanine crystal for use in the present invention also has this property.

In order to prepare a dispersion in which the crystal keeps having a small particle diameter, it is important to optimize the dispersion conditions. However, to maintain the crystal form and to prepare a dispersion including a small crystal typically establish a trade-off relationship. It is not impos-

## 16

sible to avoid the trade off, but the suitable production condition is very limited (i.e., it is very difficult to stably produce such a dispersion). Therefore, a need exists for a method by which such a dispersion as mentioned above can be easily prepared. The present inventors discover the method which is as follows.

Specifically, the method is that the titanyl phthalocyanine crystal prepared above is dispersed while applying a shear thereto an extent such that the crystal does not cause crystal change, and the dispersion is then filtered using a filter with a proper pore size. By using this method, a small amount of coarse particles (which cannot be visually observed nor detected by a particle diameter measuring instrument) can be removed from the dispersion. In addition, the particle diameter distribution of the particles in the dispersion can be properly controlled. Specifically, it is preferable to use a filter with an effective pore diameter not greater than 3  $\mu\text{m}$ , and more preferably not greater than 1  $\mu\text{m}$ . By using such a filter, a dispersion in which the titanyl phthalocyanine crystal is dispersed while having an average particle diameter not greater than 0.25  $\mu\text{m}$  (or not greater than 0.20  $\mu\text{m}$ ) can be prepared. By using this dispersion, a charge generation layer can be formed without causing coating defects. Therefore, the effects of the present invention can be fully produced.

When the dispersion to be filtered has a large average particle diameter or a wide particle diameter distribution, problems in that great loss is produced and the filtering operation cannot be performed due to clogging of the pores with coarse particles occur in the filtering process. Therefore, it is preferable that the dispersing operation is performed such that particles in the dispersion to be filtered have a particle diameter distribution such that the average particle diameter is not greater than 0.3  $\mu\text{m}$  and the standard deviation of the particle diameter is not greater than 0.2  $\mu\text{m}$ . When the average particle diameter is too large, great loss is produced. When the standard deviation is too large, the filtering operation takes a long time.

It is preferable that a proper filter is chosen depending on the size of coarse particles to be removed. As a result of the present inventors' investigation, it is found that coarse particles having a particle diameter not less than 3  $\mu\text{m}$  affect the image qualities of images with a resolution of 600 dpi (600 dots/25.4 mm). Therefore, it is preferable to use a filter with a pore diameter not greater than 3  $\mu\text{m}$ , and more preferably not greater than 1  $\mu\text{m}$ . Filters with too small a pore diameter filter out particles which can be used for the dispersion as well as coarse particles to be removed. In addition, such filters cause problems in that filtering takes a long time, the clogging problem occurs, and an excessive stress is applied to the pump used. Therefore, a filter with a proper pore diameter is preferably used. Needless to say, the filter preferably has good resistance to the solvent used for the dispersion.

By subjecting the dispersion to the filtering treatment, coarse particles can be removed from the dispersion, and thereby a charge generation layer can be formed without causing coating defects. Therefore, the resultant photoreceptor can produce high quality images without background development.

The key points in preparing the charge generation layer of the photoreceptor of the present invention are as follows:

- (1) A titanyl phthalocyanine crystal having a small particle diameter is synthesized. By using such a crystal, the dispersion time and stress applied to the crystal in the dispersing operation can be reduced, and thereby the possibility of crystal change is decreased.

(2) The content of coarse particles in the dispersion is relatively low compared to the cases where the crystal has a large particle diameter (i.e., crystals prepared by conventional methods). Therefore, a filter with a small pore diameter can be used for filtering the dispersion, and thereby coarse particles in the dispersion can be securely removed therefrom. In addition, since the amount of the particles removed from the dispersion can be decreased, the formula of the dispersion hardly changes even after the filtering process. Therefore, the desired charge generation layer can be stably produced.

(3) As a result, the photoreceptor of the present invention, which can produce high quality images without causing background development, can be stably produced.

Then the photoreceptor of the present invention will be explained referring to drawings.

FIG. 9 is a cross section of an example of the photoreceptor of the present invention. The photoreceptor has an electroconductive substrate 1, a charge blocking layer 5, a moiré preventing layer 6 and a photosensitive layer 4 including the titanyl phthalocyanine crystal which has the specific crystal form mentioned above and which has the specific average particle diameter mentioned above, wherein the layers 5, 6 and 4 are overlaid on the electroconductive substrate 1 in this order.

FIG. 10 is a cross section of another example of the photoreceptor of the present invention. The photoreceptor has an electroconductive substrate 1, a charge blocking layer 5, a moiré preventing layer 6, a charge generation layer 7 including the titanyl phthalocyanine crystal which has the specific crystal form mentioned above and which has the specific average particle diameter mentioned above, and a charge transport layer 8 including a charge transport material as a main component, wherein the layers 5, 6, 7 and 8 are overlaid on the electroconductive substrate 1 in this order.

FIG. 11 is a cross section of yet another example of the photoreceptor of the present invention. The photoreceptor has an electroconductive substrate 1, a charge blocking layer 5, a moiré preventing layer 6, a charge generation layer 7 including the titanyl phthalocyanine crystal which has the specific crystal form mentioned above and which has the specific average particle diameter mentioned above, a charge transport layer 8 including a charge transport material as a main component, and a protective layer 9, wherein the layers 5, 6, 7, 8 and 9 are overlaid on the electroconductive substrate 1 in this order.

Suitable materials for use as the electroconductive substrate 1 include materials having a volume resistivity not greater than  $10^{10} \Omega \cdot \text{cm}$ . Specific examples of such materials include plastic cylinders, plastic films or paper sheets, on the surface of which a metal such as aluminum, nickel, chromium, nichrome, copper, gold, silver, platinum and the like, or a metal oxide such as tin oxides, indium oxides and the like, is formed by deposition or sputtering. In addition, a plate of a metal such as aluminum, aluminum alloys, nickel and stainless steel can be used. A metal cylinder can also be used as the substrate 1, which is prepared by tubing a metal such as aluminum, aluminum alloys, nickel and stainless steel by a method such as impact ironing or direct ironing, and then treating the surface of the tube by cutting, super finishing, polishing and the like treatments. Further, endless belts of a metal such as nickel, stainless steel and the like can also be used as the substrate 1.

Furthermore, substrates, in which a coating liquid including a binder resin and an electroconductive powder is coated on the supports mentioned above, can be used as the substrate 1. Specific examples of such an electroconductive

powder include carbon black, acetylene black, powders of metals such as aluminum, nickel, iron, nichrome, copper, zinc, silver and the like, and metal oxides such as electroconductive tin oxides, ITO and the like. Specific examples 5 of the binder resin include known thermoplastic resins, thermosetting resins and photo-crosslinking resins, such as polystyrene, styrene-acrylonitrile copolymers, styrene-butadiene copolymers, styrene-maleic anhydride copolymers, polyesters, polyvinyl chloride, vinyl chloride-vinyl acetate 10 copolymers, polyvinyl acetate, polyvinylidene chloride, polyarylates, phenoxy resins, polycarbonates, cellulose acetate resins, ethyl cellulose resins, polyvinyl butyral resins, polyvinyl formal resins, polyvinyl toluene, poly-N-vinyl carbazole, acrylic resins, silicone resins, epoxy resins, melamine 15 resins, urethane resins, phenolic resins, alkyd resins and the like resins.

Such an electroconductive layer can be formed by coating a coating liquid in which an electroconductive powder and a binder resin are dispersed or dissolved in a proper solvent 20 such as tetrahydrofuran, dichloromethane, methyl ethyl ketone, toluene and the like solvent, and then drying the coated liquid.

In addition, substrates, in which an electroconductive resin film is formed on a surface of a cylindrical substrate 25 using a heat-shrinkable resin tube which is made of a combination of a resin such as polyvinyl chloride, polypropylene, polyesters, polyvinylidene chloride, polyethylene, chlorinated rubber and fluorine-containing resins (such as TEFILON), with an electroconductive material, can also be 30 used as the substrate 1.

Then the charge blocking layer 5 will be explained.

The function of the charge blocking layer 5 is to prevent the charges, which are induced in the electrode (i.e., the electroconductive substrate 1) and have a polarity opposite 35 to that of the voltage applied to the photoreceptor by a charger, from being injected to the photosensitive layer. Specifically, when negative charging is performed, the charge blocking layer 5 prevents injection of positive holes to the photosensitive layer. In contrast, when positive charging 40 is performed, the charge blocking layer 5 prevents injection of electrons to the photosensitive layer. Specific examples of the charge blocking layer include the following: (1) a layer prepared by anodic oxidation such as aluminum oxide layer;

- 45 (2) an insulating layer of an inorganic material such as  $\text{SiO}_2$ ;
- (3) a layer made of a network of a glassy metal oxide as disclosed in JP-A 03-191361;
- (4) a layer made of polyphosphazene as disclosed in JP-A 03-141363;
- 50 (5) a layer made of a reaction product of aminosilane as disclosed in JP-A 03-101737;
- (6) a layer made of an insulating resin; and
- (7) a crosslinked resin layer.

Among these layers, an insulating resin layer and a 55 crosslinked resin layer, which can be formed by a wet coating method, are preferably used. Since the moiré preventing layer and the photosensitive layer are typically formed on the charge blocking layer by a wet coating method, the charge blocking layer preferably has good resistance to the solvents included in the coating liquids of the moiré preventing layer and the photosensitive layer.

Suitable resins for use in the charge blocking layer include 60 thermoplastic resins such as polyamide resins, polyester resins, and vinyl chloride-vinyl acetate copolymers; and thermosetting resins which can be prepared by thermally polymerizing a compound having a plurality of active hydrogen atoms (such as hydrogen atoms of  $-\text{OH}$ ,  $-\text{NH}_2$ ,

and —NH) with a compound having a plurality of isocyanate groups and/or a compound having a plurality of epoxy groups.

Specific examples of the compounds having a plurality of active hydrogen atoms include polyvinyl butyral, phenoxy resins, phenolic resins, polyamide resins, phenolic resins, polyamide resins, polyester resins, polyethylene glycol resins, polypropylene glycol resins, polybutylene glycol resins, and acrylic resins (such as hydroxyethyl methacrylate resins). Specific examples of the compounds having a plurality of isocyanate groups include tolylene diisocyanate, hexamethylene diisocyanate, diphenylmethane diisocyanate, and prepolymers thereof. Specific examples of the compounds having a plurality of epoxy groups include bisphenol A based epoxy resins, etc.

Among these resins, polyamide resins are preferably used in view of film formability, environmental stability and resistance to solvents.

In addition, oil-free alkyd resins; amino resins such as thermosetting amino resins prepared by thermally polymerizing a butylated melamine resin; and photo-crosslinking resins prepared by reacting an unsaturated resin, such as unsaturated polyurethane resins unsaturated polyester resins, with a photo-polymerization initiator such as thioxanthone compounds and methylbenzyl formate, can also be used.

In addition, electroconductive polymers having a rectification property, and layers including a resin or a compound having an electron accepting or donating property which is determined depending on the polarity of the charges formed on the surface of the photoreceptor can also be used.

The charge blocking layer 5 preferably has a thickness not less than 0.1  $\mu\text{m}$  and less than 2.0  $\mu\text{m}$ , and more preferably from 0.3  $\mu\text{m}$  to 1.0  $\mu\text{m}$ . When the charge blocking layer is too thick, the residual potential of the photoreceptor increases after imagewise light irradiation is repeatedly performed particularly under low temperature and low humidity conditions. In contrast, the charge blocking layer is too thin, the charge blocking effect is hardly produced. The charge blocking layer 5 can include one or more materials such as crosslinking agents, solvents, additives and crosslinking promoters. The charge blocking layer 5 can be prepared by coating a coating liquid by a coating method such as blade coating, dip coating, spray coating, bead coating and nozzle coating, followed by drying and crosslinking using heat or light.

Then the moiré preventing layer 6 will be explained.

The function of the moiré preventing layer 6 is to prevent occurrence of moiré in the resultant images due to interference of light, which is caused when coherent light (such as laser light) is used for optical writing. Namely, the moiré preventing layer scatters the light used for optical writing. In order to carry out this function, the layer preferably includes a material having a high refractive index. The moiré preventing layer typically includes a binder resin and an inorganic pigment. Suitable inorganic pigments include white inorganic pigments. Specific examples of the white inorganic pigments include titanium oxide, calcium fluoride, calcium oxide, silica, magnesium oxide and aluminum oxide. Among these pigments, titanium oxide is preferably used because of having high hiding power.

As can be understood from FIGS. 9-11, injection of charges from the substrate 1 is blocked by the charge blocking layer 5 and therefore the moiré preventing layer 6 preferably has an ability to transport charges having the same polarity as that of the charges formed on the surface of the photoreceptor, to prevent increase of residual potential.

For example, in a case of a negative charge type photoreceptor, the moiré preventing layer 6 preferably has an electron conducting ability. Therefore it is preferable to use an electroconductive inorganic pigment or a conductive inorganic pigment for the moiré preventing layer 6. Alternatively, an electroconductive material (such as acceptors) may be added to the moiré preventing layer 6.

Specific examples of the binder resin for use in the moiré preventing layer 6 include the resins mentioned above for 10 use in the charge blocking layer 5. Since the photosensitive layer 4 is formed on the moiré preventing layer 6 by coating a coating liquid, the binder resin preferably has a good resistance to the solvent included in the photosensitive layer coating liquid. Among the resins, thermosetting resins, and 15 more preferably mixtures of alkyd and melamine resins, are preferably used as the binder resin of the moiré preventing layer 6. The mixing ratio of an alkyd resin to a melamine resin is an important factor influencing the structure and properties of the moiré preventing layer 6, and the weight 20 ratio thereof is preferably from 5/5 to 8/2. When the content of melamine resin is too high, the coated film is shrunk in the thermosetting process, and thereby coating defects are formed in the resultant film. In addition, the residual potential increasing problem occurs. In contrast, when the content of alkyd resin is too high, the electric resistance of the layer seriously decreases, and thereby the resultant images have background fouling, although the residual potential of the photoreceptor is reduced.

The mixing ratio of the inorganic pigment to the binder 30 resin in the moiré preventing layer 6 is also an important factor, and the volume ratio thereof is preferably from 1/1 to 3/1. When the ratio is too low (i.e., the content of the inorganic pigment is too low), not only the moiré preventing effect deteriorates but also the residual potential increases 35 after repeated use. In contrast, when the ratio is too high, the film formability of the layer deteriorates, resulting in deterioration of surface conditions of the resultant layer. In addition, a problem in that the upper layer (e.g., the photosensitive layer) cannot form a good film thereon because the 40 coating liquid penetrates into the moiré preventing layer occurs. This problem is fatal to the photoreceptor having a layered photosensitive layer including a thin charge generation layer as a lower layer because such a thin charge generation layer cannot be formed on such a moiré preventing layer. In addition, when the ratio is too large, a problem 45 in that the surface of the inorganic pigment cannot be covered with the binder resin. In this case, the charge generation material is directly contacted with the inorganic pigment and thereby the possibility of occurrence of a problem in that carriers are thermally produced increases, resulting in occurrence of the background development problem.

By using two kinds of titanium oxides having different 50 average particle diameters for the moiré preventing layer, the substrate 1 is effectively hidden by the moiré preventing layer and thereby occurrence of moiré fringes can be well 55 prevented and formation of pinholes in the layer can also be prevented. In this regard, the average particle diameters (D1 and D2) of the two kinds of titanium oxides preferably 60 satisfy the following relationship:

$$0.2 < D2/D1 \leq 0.5.$$

When the ratio D2/D1 is too low, the surface of the titanium oxide becomes more active, and thereby stability of the electrostatic properties of the resultant photoreceptor seriously deteriorates. In contrast, when the ratio is too high, the electroconductive substrate 1 cannot be well hidden by

the moiré preventing layer and thereby the moiré preventing effect deteriorates and abnormal images such as moiré fringes are produced. In this regard, the average particle diameter of the pigment means the average particle diameter of the pigment in a dispersion prepared by dispersing the pigment in water while applying a strong shear force thereto.

Further, the average particle diameter (D2) of the titanium oxide (T2) having a smaller average particle diameter is also an important factor, and is preferably from 0.05  $\mu\text{m}$  to 0.20  $\mu\text{m}$ . When D2 is too small, hiding power of the layer deteriorates. Therefore, moiré fringes tend to be caused. In contrast, when D2 is too large, the filling factor of the titanium oxide in the layer is small, and thereby background development preventing effect cannot be well produced.

The mixing ratio of the two kinds of titanium oxides in the moiré preventing layer **6** is also an important factor, and is preferably determined such that the following relationship is satisfied:

$$0.2 \leq T2/(T1+T2) \leq 0.8,$$

wherein T1 represents the weight of the titanium oxide having a larger average particle diameter, and T2 represents the weight of the titanium oxide having a smaller average particle diameter.

When the mixing ratio is too low, the filling factor of the titanium oxide in the layer is small, and thereby background development preventing effect cannot be well produced. In contrast, when the mixing ratio is too high, the hiding power of the layer deteriorates, and thereby the moiré preventing effect cannot be well produced.

The moiré preventing layer preferably has a thickness of from 1 to 10  $\mu\text{m}$ , and more preferably from 2 to 5  $\mu\text{m}$ . When the layer is too thin, the moiré preventing effect cannot be well produced. In contrast, when the layer is too thick, the residual potential increases.

The moiré preventing layer is typically prepared as follows. An inorganic pigment is dispersed in a solvent together with a binder resin using a dispersion machine such as ball mills, sand mills, and attritors. In this case, crosslinking agents, other solvents, additives, crosslinking promoters, etc., can be added thereto if desired. The thus prepared coating liquid is coated on the charge blocking layer by a method such as blade coating, dip coating, spray coating, bead coating and nozzle coating, followed by drying and crosslinking using light or heat.

Then the photosensitive layer **4** will be explained.

The photosensitive layer **4** may be a single-layered photosensitive layer including a charge generation material and a charge transport material. However, the photosensitive layer **4** is preferably a multi-layered photosensitive layer including the charge generation layer **7** and the charge transport layer **8** because of having good photosensitivity and good durability.

The charge generation layer **7** includes the titanyl phthalocyanine crystal which has an average primary particle diameter not greater than 0.25  $\mu\text{m}$  and includes no coarse particles and which has an X-ray diffraction spectrum such that a maximum peak is observed at a Bragg (20) angle of  $27.2 \pm 0.2^\circ$  a peak is observed at Bragg (20) angle of  $9.4 \pm 0.2^\circ$ ,  $9.6 \pm 0.2^\circ$  and  $24.0 \pm 0.2^\circ$ ; a lowest angle peak is observed at an angle of  $7.3 \pm 0.2^\circ$ ; no peak is observed between the lowest angle peak and the  $9.4^\circ$  peak; and no peak is observed at a Bragg (20) angle of  $26.3 \pm 0.2^\circ$ , when a Cu—K $\alpha$  X-ray having a wavelength of 1.542  $\text{\AA}$  is used.

The charge generation layer **7** is typically prepared by coating a coating liquid, which is prepared by dispersing the

titanyl phthalocyanine pigment in a solvent, optionally together with a binder resin, using a ball mill, an attritor, a sand mill or an ultrasonic dispersion machine, followed by drying. Suitable coating methods include dip coating, spray coating, bead coating, nozzle coating, spinner coating and ring coating.

Specific examples of the binder resins, which are optionally included in the charge generation layer coating liquid, include polyamide, polyurethane, epoxy resins, polyketone, polycarbonate, silicone resins, acrylic resins, polyvinyl butyral, polyvinyl formal, polyvinyl ketone, polystyrene, polysulfone, poly-N-vinylcarbazole, polyacrylamide, polyvinyl benzal, polyester, phenoxy resins, vinyl chloride-vinyl acetate copolymers, polyvinyl acetate, polyphenylene oxide, polyamides, polyvinyl pyridine, cellulose resins, casein, polyvinyl alcohol, polyvinyl pyrrolidone, and the like resins.

The content of the binder resin in the charge generation layer is preferably from 0 to 500 parts by weight, and preferably from 10 to 300 parts by weight, per 100 parts by weight of the charge generation material included in the layer.

Specific examples of the solvents for use in the charge generation layer coating liquid include isopropanol, acetone, methyl ethyl ketone, cyclohexanone, tetrahydrofuran, dioxane, ethyl cellosolve, ethyl acetate, methyl acetate, dichloromethane, dichloroethane, monochlorobenzene, cyclohexane, toluene, xylene, ligroin, and the like solvents.

The charge generation layer preferably has a thickness of from 0.01 to 5  $\mu\text{m}$ , and more preferably from 0.1 to 2  $\mu\text{m}$ .

Then the charge transport layer **8** will be explained. The charge transport layer **8** is typically prepared by coating a coating liquid, which is prepared by dissolving or dispersing a charge transport material in a solvent optionally together with a binder resin, followed by drying. If desired, additives such as plasticizers, leveling agents and antioxidants can be added to the coating liquid.

Charge transport materials are classified into positive-hole transport materials and electron transport materials.

Specific examples of the positive-hole transport materials include known materials such as poly-N-vinyl carbazole and its derivatives, poly- $\gamma$ -carbazolylethylglutamate and its derivatives, pyrene-formaldehyde condensation products and their derivatives, polyvinyl pyrene, polyvinyl phenanthrene, polysilane, oxazole derivatives, oxadiazole derivatives, imidazole derivatives, monoarylamines, diarylamines, triarylamines, stilbene derivatives,  $\alpha$ -phenyl stilbene derivatives, benzidine derivatives, diarylmethane derivatives, triaryl methane derivatives, 9-styrylanthracene derivatives, pyrazoline derivatives, divinyl benzene derivatives, hydrazone derivatives, indene derivatives, butadiene derivatives, pyrene derivatives, bisstilbene derivatives, enamine derivatives, and the like.

Specific examples of the electron transport materials include electron accepting materials such as chloranil, bromanil, tetracyanoethylene, tetracyanoquinoxidimethane, 2,4,7-trinitro-9-fluorenol, 2,4,5,7-tetrinitro-9-fluorenol, 2,4,5,7-tetranitroanthrone, 2,4,8-trinitrothioxanthone, 2,6,8-trinitro-4H-indeno[1,2-b]thiophene-4-one, 1,3,7-trinitro dibenzothiophene-5,5-dioxide, benzoquinone derivatives and the like.

These charge transport materials can be used alone or in combination.

Specific examples of the binder resin for use in the charge transport layer include known thermoplastic resins and thermosetting resins, such as polystyrene, styrene-acrylonitrile copolymers, styrene-butadiene copolymers, styrene-maleic anhydride copolymers, polyester, polyvinyl chloride,

23

vinyl chloride-vinyl acetate copolymers, polyvinyl acetate, polyvinylidene chloride, polyarylate, phenoxy resins, polycarbonate, cellulose acetate resins, ethyl cellulose resins, polyvinyl butyral resins, polyvinyl formal resins, polyvinyl toluene, poly-N-vinyl carbazole, acrylic resins, silicone resins, epoxy resins, melamine resins, urethane resins, phenolic resins, alkyd resins and the like.

The content of the charge transport material in the charge transport layer is preferably from 20 to 300 parts by weight, and more preferably from 40 to 150 parts by weight, per 100 parts by weight of the binder resin included in the charge transport layer. The thickness of the charge transport layer **8** is preferably from 5 to 100  $\mu\text{m}$ .

Suitable solvents for use in the charge transport layer coating liquid include tetrahydrofuran, dioxane, toluene, dichloromethane, monochlorobenzene, dichloroethane, cyclohexanone, methyl ethyl ketone, acetone and the like solvents. In view of environmental protection, non-halogenated solvents are preferably used. Specifically, cyclic ethers such as tetrahydrofuran, dioxolan and dioxane, aromatic hydrocarbons such as toluene and xylene, and their derivatives are preferably used.

Charge transport polymers, which have both a binder resin function and a charge transport function, can be preferably used for the charge transport layer because the resultant charge transport layer has good abrasion resistance.

Suitable charge transport polymers include known charge transport polymer materials. Among these materials, polycarbonate resins having a triarylamine group in their main chain and/or side chain are preferably used. In particular, charge transport polymers having the following formulae of from (1) to (10) are preferably used:



wherein  $R_1$ ,  $R_2$  and  $R_3$  independently represent a substituted or unsubstituted alkyl group, or a halogen atom;  $R_4$  represents a hydrogen atom, or a substituted or unsubstituted alkyl group;  $R_5$ , and  $R_6$  independently represent a substituted or unsubstituted aryl group;  $r$ ,  $p$  and  $q$  independently represent 0 or an integer of from 1 to 4;  $k$  is a number of from 0.1 to 1.0 and  $j$  is a number of from 0 to 0.9;  $n$  is an integer of from 5 to 5000; and  $X$  represents a divalent aliphatic group, a divalent alicyclic group or a divalent group having the following formula:



24

wherein  $R_{101}$  and  $R_{102}$  independently represent a substituted or unsubstituted alkyl group, a substituted or unsubstituted aryl group, or a halogen atom;  $t$  and  $m$  represent 0 or an integer of from 1 to 4;  $v$  is 0 or 1; and  $Y$  represents a linear alkylene group, a branched alkylene group, a cyclic alkylene group,  $-\text{O}-$ ,  $-\text{S}-$ ,  $-\text{SO}-$ ,  $-\text{SO}_2-$ ,  $-\text{CO}-$ ,  $-\text{CO}-\text{O}-\text{Z}-\text{O}-\text{CO}$  ( $Z$  represents a divalent aliphatic group), or a group having the following formula:



wherein  $a$  is an integer of from 1 to 20;  $b$  is an integer of from 1 to 2000; and  $R_{103}$  and  $R_{104}$  independently represent a substituted or unsubstituted alkyl group, or a substituted or unsubstituted aryl group, wherein  $R_{101}$ ,  $R_{102}$ ,  $R_{103}$  and  $R_{104}$  may be the same or different from the others.



wherein  $R_7$  and  $R_8$  independently represent a substituted or unsubstituted aryl group;  $Ar_1$ ,  $Ar_2$  and  $Ar_3$  independently represent an arylene group; and  $X$ ,  $k$ ,  $j$  and  $n$  are defined above in formula (1).



25

wherein  $R_9$  and  $R_{10}$  independently represent a substituted or unsubstituted aryl group;  $Ar_4$ ,  $Ar_5$  and  $Ar_6$  independently represent an arylene group; and  $X$ ,  $k$ ,  $j$  and  $n$  are defined above in formula (1).



wherein  $R_{11}$  and  $R_{12}$  independently represent a substituted or unsubstituted aryl group;  $Ar_7$ ,  $Ar_8$  and  $Ar_9$  independently represent an arylene group;  $p$  is an integer of from 1 to 5; and  $X$ ,  $k$ ,  $j$  and  $n$  are defined above in formula (1).



wherein  $R_{13}$  and  $R_{14}$  independently represent a substituted or unsubstituted aryl group;  $Ar_{10}$ ,  $Ar_{11}$  and  $Ar_{12}$  independently represent an arylene group;  $X_1$  and  $X_2$  independently represent a substituted or unsubstituted ethylene group, or a substituted or unsubstituted vinylene group; and  $X$ ,  $k$ ,  $j$  and  $n$  are defined above in formula (1).

alkylene group, a substituted or unsubstituted cycloalkylene group, a substituted or unsubstituted alkyleneether group, an oxygen atom, a sulfur atom, or a vinylene group;  $u$ ,  $v$  and  $w$  independently represent 0 or 1; and  $X$ ,  $k$ ,  $j$  and  $n$  are defined above in formula (1).



wherein  $R_{15}$ ,  $R_{16}$ ,  $R_{17}$  and  $R_{18}$  independently represent a substituted or unsubstituted aryl group;  $Ar_{13}$ ,  $Ar_{14}$ ,  $Ar_{15}$  and  $Ar_{16}$  independently represent an arylene group;  $Y_1$ ,  $Y_2$  and  $Y_3$  independently represent a substituted or unsubstituted



wherein  $R_{19}$  and  $R_{20}$  independently represent a hydrogen atom, or substituted or unsubstituted aryl group, and  $R_{19}$  and  $R_{20}$  optionally share bond connectivity to form a ring;  $Ar_{17}$ ,  $Ar_{18}$  and  $Ar_{19}$  independently represent an arylene group; and  $X$ ,  $k$ ,  $j$  and  $n$  are defined above in formula (1).



wherein  $R_{21}$  represents a substituted or unsubstituted aryl group;  $Ar_{20}$ ,  $Ar_{21}$ ,  $Ar_{22}$  and  $Ar_{23}$  independently represent an arylene group; and  $X$ ,  $k$ ,  $j$  and  $n$  are defined above in formula (1).



wherein  $R_{22}$ ,  $R_{23}$ ,  $R_{24}$  and  $R_{25}$  independently represent a substituted or unsubstituted aryl group;  $Ar_{24}$ ,  $Ar_{25}$ ,  $Ar_{26}$ ,  $Ar_{27}$  and  $Ar_{28}$  independently represent an arylene group; and  $X$ ,  $k$ ,  $j$  and  $n$  are defined above in formula (1).



wherein  $R_{26}$  and  $R_{27}$  independently represent a substituted or unsubstituted aryl group;  $Ar_{29}$ ,  $Ar_{30}$  and  $Ar_{31}$  independently represent an arylene group; and  $X$ ,  $k$ ,  $j$  and  $n$  are defined above in formula (1).

Formulae (1) to (10) are illustrated in the form of block copolymers, but the polymers are not limited thereto, and may be random copolymers.

In addition, the charge transport layer can also be formed by coating one or more monomers or oligomers, which have an electron donating group, and then subjecting the monomers or oligomers to a crosslinking reaction after forming the layer such that the layer has a two- or three-dimensional structure.

Further, the charge transport layer can be constituted of a layer having a crosslinked structure. The crosslinked structure can be formed, for example, by performing a crosslinking reaction using one or more reactive monomers having a plurality of crosslinkable functional groups in their molecule and using light or heat energy, resulting in formation of three-dimensional network structure. When the charge transport layer has such a structure, the photoreceptor has good abrasion resistance. In this case, it is preferable to use one or more monomers having a charge transportability as the reactive monomers. By using such monomers, the resultant network structure has a charge transport moiety therein, and therefore the layer has good charge transportability. Suitable monomers for use as the monomers having a charge transportability include reactive monomers having a triarylamine structure.

The charge transport layer having such a crosslinked structure reduces its volume when crosslinked. Therefore,

when such a charge transport layer is formed while having too large a thickness, a problem in that the layer has a crack occurs. Therefore it is preferable to form a layered charge transport layer which includes a lower charge transport layer including a polymer and a low molecular weight charge transport material and an upper charge transport layer including such a crosslinked charge transport layer.

The charge transport layer constituted of a polymer or a crosslinked polymer, which has an electron donating group, has good abrasion resistance. In electrophotographic image forming apparatus, the potential of the charges formed on a photoreceptor (i.e., the potential of a non-lighted area) is generally set to be constant. Therefore, the larger the abrasion amount of the photosensitive layer of the photoreceptor, the larger the electric field formed on the photoreceptor.

When the electric field increases, background development occurs in the resultant images. Namely a photoreceptor having good abrasion resistance hardly causes the background development problem. The above-mentioned charge 20 transport layer constituted of a polymer having an electron donating group has good film formability because the layer itself a polymer. In addition, the charge transport layer has good charge transportability because of including charge transport moieties at a relatively high concentration compared to charge transport layers including a polymer and a low molecular weight charge transport material. Namely, the photoreceptor including a charge transport layer constituted of a charge transport polymer has high response.

Known copolymers, block polymers, graft polymers, and star polymers can also be used for the polymers having an electron donating group. In addition, crosslinking polymers including an electron donating group, which have been disclosed in JP-As 03-109406, 2000-206723, and 2001-34001, can also be used for the charge transport layer.

35 The charge transport layer may include additives such as plasticizers and leveling agents. Specific examples of the plasticizers include known plasticizers such as dibutyl phthalate and dioctyl phthalate. The content of the plasticizer in the CTL is from 0 to 30% by weight based on the  
40 binder resin included in the charge transport layer. Specific examples of the leveling agents include silicone oils such as dimethyl silicone oils and methyl phenyl silicone oils, and polymers and oligomers, which include a perfluoroalkyl group in their side chain. The content of the leveling agent  
45 in the CTL is from 0 to 1% by weight based on the binder resin included in the charge transport layer.

Hereinbefore, the layered photosensitive layer is explained. However, the photosensitive layer of the photoreceptor of the present invention is not limited to the layered photosensitive layer, and a single-layered photosensitive layer can be used. In this case, the photosensitive layer 4 includes at least a charge generation material and a binder resin. Suitable materials for use as the binder resin include the materials mentioned above for use as the binder resin in the charge generation layer and charge transport layer. In addition, a charge transport material is preferably added to the single-layered photosensitive layer so that the resultant photoreceptor has high photosensitivity, high carrier transportability and low residual potential. In this case, a proper charge transport material is chosen from hole transport materials or electron transport materials of the charge transport materials which is determined depending on the charges to be formed on the surface of the photoreceptor. In addition, the charge transport polymers mentioned above can also be preferably used for the single-layered photosensitive layer.

In the photoreceptor of the present invention, a protective layer 9 is optionally formed on the photosensitive layer to

protect the photosensitive layer. Recently, computers are used in daily life, and therefore a need exists for a high-speed and small-sized printer. By forming a protective layer on the photosensitive layer, the resultant photoreceptor has good durability while having a high sensitivity and producing images without abnormal images.

Specific examples of the material for use in the protective layer 9 include ABS resins, ACS resins, olefin-vinyl monomer copolymers, chlorinated polyether, aryl resins, phenolic resins, polyacetal, polyamide, polyamideimide, polylysulfone, polybutylene, polybutyleneterephthalate, polycarbonate, polyarylate, polyethersulfone, polyethylene, polyethyleneterephthalate, polyimide, acrylic resins, polymethylpentene, polypropylene, polyphenyleneoxide, polysulfone, polystyrene, AS resins, butadiene-styrene copolymers, polyurethane, polyvinyl chloride, polyvinylidene chloride, epoxy resins, etc. Among these resins, polycarbonate and polyarylate are preferably used.

In addition, in order to impart good abrasion resistance to the protective layer, fluorine-containing resins such as polytetrafluoroethylene, and silicone resins can be used therefor. Further, combinations of such resins and an inorganic filler such as titanium oxide, aluminum oxide, tin oxide, zinc oxide, zirconium oxide, magnesium oxide, potassium titanate and silica or an organic filler can also be used therefor. These inorganic fillers may be subjected to a surface treatment.

In addition, organic and inorganic fillers can be used in the protective layer. Suitable organic fillers include powders of fluorine-containing resins such as polytetrafluoroethylene, silicone resin powders, amorphous carbon powders, etc. Specific examples of the inorganic fillers include powders of metals such as copper, tin, aluminum and indium; metal oxides such as alumina, silica, tin oxide, zinc oxide, titanium oxide, alumina, zirconia, indium oxide, antimony oxide, bismuth oxide, calcium oxide, tin oxide doped with antimony, indium oxide doped with tin; potassium titanate, etc. In view of hardness, the inorganic fillers are preferable. In particular, silica, titanium oxide and alumina are preferable.

The content of the filler in the protective layer is preferably determined depending on the species of the filler used and the application of the resultant photoreceptor, but the content of a filler in the surface portion of the protective layer is preferably not less than 5% by weight, more preferably from 10 to 50% by weight, and even more preferably from 10 to 30% by weight, based on the total weight of the surface portion of the protective layer.

The filler included in the protective layer preferably has a volume average particle diameter of from 0.1 to 2  $\mu\text{m}$ , and more preferably from 0.3 to 1  $\mu\text{m}$ . When the average particle diameter is too small, good abrasion resistance cannot be imparted to the resultant photoreceptor. In contrast, when the average particle diameter is too large, the surface of the resultant protective layer is seriously roughened or a problem such that a protective layer itself cannot be formed occurs.

In the present application, the average particle diameter of a filler means a volume average particle diameter unless otherwise specified, and is measured using an instrument, CAPA-700 manufactured by Horiba Ltd. In this case, the cumulative 50% particle diameter (i.e., the median particle diameter) is defined as the average particle diameter. In addition, it is preferable that the standard deviation of the particle diameter distribution curve of the filler used in the protective layer is not greater than 1  $\mu\text{m}$ . When the standard deviation is too large (i.e., when the filler has too broad

particle diameter distribution), the effect of the present invention cannot be produced.

The pH of the filler used in the protective layer coating liquid largely influences on the dispersibility of the filler therein and the resolution of the images produced by the resultant photoreceptor. The reasons therefor are as follows. Fillers (in particular, metal oxides) typically include hydrochloric acid therein which is used during the production of the fillers. When the residual amount of hydrochloric acid is large, the resultant photoreceptor tends to produce blurred images. In addition, inclusion of too large an amount of hydrochloric acid causes the dispersibility of the filler to deteriorate.

Another reason therefor is that the charge properties of fillers (in particular, metal oxides) are largely influenced by the pH of the fillers. In general, particles dispersed in a liquid are charged positively or negatively. In this case, ions having a charge opposite to the charge of the particles gather around the particles to neutralize the charge of the particles, resulting in formation of an electric double layer, and thereby the particles are stably dispersed in the liquid. The potential (i.e., zeta potential) of a point around one of the particles decreases (i.e., approaches to zero) as the distance between the point and the particle increases. Namely, a point far apart from the particle is electrically neutral, i.e., the zeta potential thereof is zero. In this case, the higher the zeta potential, the better the dispersion of the particles. When the zeta potential is nearly equal to zero, the particles easily aggregate. The zeta potential of a system largely depends on the pH of the system. When the system has a certain pH, the zeta potential becomes zero. This point is called an isoelectric point. It is preferable to increase the zeta potential by setting the pH of the system to be far apart from the isoelectric point, in order to stabilize the dispersion of the system.

It is preferable for the protective layer to include a filler having a pH of 5 or more at the isoelectric point, in order to prevent formation of blurred images. In other words, fillers having a highly basic property can be preferably used in the photoreceptor of the present invention because the effect of the present invention can be heightened. Fillers having a highly basic property have a high zeta potential (i.e., the fillers are stably dispersed) when the system for which the fillers are used is acidic.

In this application, the pH of a filler means the pH of the filler at the isoelectric point, which is determined by the zeta potential of the filler. Zeta potential can be measured by a laser beam potential meter manufactured by Ootsuka Electric Co., Ltd.

In addition, in order to prevent production of blurred images, fillers having a high electric resistance (i.e., not less than  $1 \times 10^{10} \Omega\cdot\text{cm}$  in resistivity) are preferably used. Further, fillers having a pH not less than 5 and fillers having a dielectric constant not less than 5 can be more preferably used. Fillers having a dielectric constant not less than 5 and/or a pH not less than 5 can be used alone or in combination. In addition, combinations of a filler having a pH not less than 5 and a filler having a pH less than 5, or combinations of a filler having a dielectric constant not less than 5 and a filler having a dielectric constant less than 5, can also be used. Among these fillers,  $\alpha$ -alumina having a closest packing structure is preferably used. This is because  $\alpha$ -alumina has a high insulating property, a high heat stability and a good abrasion resistance, resulting in prevention of formation of blurred images and improvement of abrasion resistance of the resultant photoreceptor.

In the present application, the resistivity of a filler is defined as follows. The resistivity of a powder such as fillers

largely changes depending on the filling factor of the powder when the resistivity is measured. Therefore, it is necessary to measure the resistivity under a constant condition. In the present application, the resistivity is measured by a device similar to the devices disclosed in JP-As 5-94049 and 5-113688. The surface area of the electrodes of the device is 4.0 cm<sup>2</sup>. Before the resistivity of a sample powder is measured, a load of 4 kg is applied to one of the electrodes for 1 minute and the amount of the sample powder is adjusted such that the distance between the two electrodes becomes 4 mm.

The resistivity of the sample powder is measured by pressing the sample powder only by the weight (i.e., 1 kg) of the upper electrode without applying any other load to the sample. The voltage applied to the sample powder is 100 V. When the resistivity is not less than 10<sup>6</sup> Ω·cm, HIGH RESISTANCE METER (from Yokogawa Hewlett-Packard Co.) is used to measure the resistivity. When the resistivity is less than 10<sup>6</sup> Ω·cm, a digital multimeter (from Fluke Corp.) is used.

The dielectric constant of a filler is measured as follows. A cell similar to that used for measuring the resistivity is also used for measuring the dielectric constant. After a load is applied to a sample powder, the capacity of the sample powder is measured using a dielectric loss measuring instrument (from Ando Electric Co., Ltd.) to determine the dielectric constant of the powder.

The fillers to be included in the protective layer are preferably subjected to a surface treatment using a surface treatment agent in order to improve the dispersion of the fillers in the protective layer. When a filler is poorly dispersed in the protective layer, the following problems occur.

- (1) the residual potential of the resultant photoreceptor increases;
- (2) the transparency of the resultant protective layer decreases;
- (3) coating defects are formed in the resultant protective layer;
- (4) the abrasion resistance of the protective layer deteriorates;
- (5) the durability of the resultant photoreceptor deteriorates; and
- (6) the image qualities of the images produced by the resultant photoreceptor deteriorate.

Suitable surface treatment agents include known surface treatment agents. However, surface treatment agents which can maintain the highly insulative property of the fillers used are preferably used.

As the surface treatment agents, titanate coupling agents, aluminum coupling agents, zirconium coupling agents, higher fatty acids, combinations of these agents with a silane coupling agent, Al<sub>2</sub>O<sub>3</sub>, TiO<sub>2</sub>, ZrO<sub>2</sub>, silicones, aluminum stearate, and the like, can be preferably used to improve the dispersibility of fillers and to prevent formation of blurred images. These materials can be used alone or in combination.

When fillers treated with a silane coupling agent are used, the resultant photoreceptor tends to produce blurred images. However, combinations of a silane coupling agent with one of the surface treatment agents mentioned above can often produce good images without blurring.

The coating weight of the surface treatment agents is preferably from 3 to 30% by weight, and more preferably from 5 to 20% by weight, based on the weight of the treated filler although the weight is determined depending on the average primary particle diameter of the filler.

When the content of the surface treatment agent is too low, the dispersibility of the filler cannot be improved. In contrast, when the content is too high, the residual potential of the resultant photoreceptor seriously increases.

These fillers can be dispersed using a proper dispersion machine. In this case, the fillers are preferably dispersed such that the aggregated particles are dissociated and primary particles are dispersed to improve the transparency of the resultant protective layer.

In addition, a charge transport material can be included in the protective layer to enhance the photo response and to reduce the residual potential of the resultant photoreceptor. The charge transport materials mentioned above for use in the charge transport layer can also be used for the protective layer.

When a low molecular weight charge transport material is used for the protective layer, the concentration of the charge transport material may be changed in the thickness direction of the protective layer. Specifically, it is preferable to reduce

the concentration of the charge transport material at the surface portion of the protective layer in order to improve the abrasion resistance of the resultant photoreceptor. At this point, the concentration of the charge transport material means the ratio of the weight of the charge transport material to the total weight of the protective layer.

It is preferable to use a charge transport polymer in the protective layer in order to improve the durability of the photoreceptor.

The protective layer 9 can be formed by any known coating methods. The thickness of the protective layer is preferably from 1 to 10 μm. In addition, layers of amorphous carbon or amorphous silicon carbide, which are formed by a vacuum deposition method, can also be used as the protective layer 9.

Then the image forming apparatus of the present invention will be explained in detail.

FIG. 12 is a schematic view illustrating an embodiment of the image forming apparatus of the present invention.

Referring to FIG. 12, a photoreceptor 11 is the photoreceptor of the present invention, which includes at least an electroconductive substrate, and a charge blocking layer, a moiré preventing layer, and a photosensitive layer, which are located overlying the electroconductive substrate in this order, wherein the photosensitive layer includes a titanyl

phthalocyanine crystal which has an average primary particle diameter not greater than 0.25 μm and has an X-ray diffraction spectrum such that a maximum peak is observed at a Bragg (20) angle of 27.2°±0.2°; a peak is observed at Bragg (20) angle of 9.4°±0.2°, 9.6±0.2° and 24.0±0.2°; a lowest angle peak is observed at an angle of 7.3°±0.2°; no peak is observed between the lowest angle peak and the 9.4° peak; and no peak is observed at a Bragg (20) angle of 26.3°±0.2°, when a Cu—Kα X-ray having a wavelength of 1.542 Å is used.

The photoreceptor has a cylindrical form, but sheet-form photoreceptors and endless belt-form photoreceptors can also be used.

Around the photoreceptor 11, a quenching lamp 12 configured to discharge the charges remaining on the photoreceptor 12, a charger 13 configured to charge the photoreceptor 11, an imagewise light irradiator 15 configured to irradiate the photoreceptor 11 with imagewise light to form an electrostatic latent image on the photoreceptor 11, an image developer 16 configured to develop the latent image with a toner to form a toner image on the photoreceptor 11, and a cleaning unit including a cleaning brush 24 and a cleaning blade 25 configured to clean the surface of the

33

photoreceptor 11 are arranged while contacting or being set closely to the photoreceptor 11. The toner image formed on the photoreceptor 11 is transferred on a receiving paper 19 fed by a pair of registration rollers 18 at a transfer device (i.e., a pair of a transfer charger 20 and a separating charger 21). The receiving paper 19 having the toner image thereon is separated from the photoreceptor 11 by a separating pick 22.

In the image forming apparatus of the present invention, a pre-transfer charger 17 and a pre-cleaning charger 23 may be arranged if desired.

As the charger 13, the pre-transfer charger 17, the transfer charger 20, the separating charger 21 and the pre-cleaning charger 23, all known chargers such as corotrons, scorotrons, solid state chargers, roller chargers and brush chargers can be used.

As the charging devices, contact chargers such as charging rollers, charging blades and charging brushes and short-range chargers which charge a photoreceptor while a small gap is formed between the charging member and the photoreceptor can be preferably used. In particular, by using contact chargers, the amount of generated ozone can be drastically reduced, and therefore the photoreceptor can be maintained to be stable and deterioration of image qualities can be prevented even when the photoreceptor is repeatedly used. In addition, the image forming apparatus can be minimized in size.

Among the contact chargers, charging rollers and charging brushes can be preferably used in the present invention.

In the short-range chargers for use in the image forming apparatus of the present invention, the gap between the proximity charging member and the photoreceptor is about 100  $\mu\text{m}$ , and therefore the short-range chargers are different from known non-contact chargers such as corotrons and scorotrons. Any mechanisms which can maintain such a small gap between the surface of the charging member and the surface of the photoreceptor to be charged, can be used for the short-range chargers for use in the image forming apparatus of the present invention. For example, mechanisms having a constitution such that a proper gap is formed between the surface of the photoreceptor and the surface of the charging member by mechanically fixing the rotation shaft of the photoreceptor to the rotation shaft of the charging member can be used. Among these mechanisms, the following is preferable:

- (1) A charger having a gap forming member on both sides thereof is provided. The gap forming members contact the non-image areas of the photoreceptor to form a proper gap therebetween; and
- (2) Gap forming members are provided on the non-image areas of the photoreceptor. The image forming members contact the non-image forming areas of a charger to form a proper gap therebetween.

In particular, short-range chargers disclosed in JP-As. 2002-148904 and 2002-148905 are preferably used in the image forming apparatus of the present invention.

FIG. 13 is a schematic view illustrating an embodiment of the short-range charger for use in the image forming apparatus of the present invention, in which a gap forming member is formed on a charger. Referring to FIG. 13, numerals 11 and 13 designate the photoreceptor and charging roller, respectively. Numerals 31, 32, 33 and 34 designate a gap forming member, a metal shaft of the charging roller, an image forming area of the photoreceptor 11, and non-image areas of the photoreceptor 11, respectively. The gap forming members 31 contact the non-image areas 34 of

34

the photoreceptor 11 to form a gap between the image forming area 33 and the charging area of the charging roller 13.

The above-mentioned short-range charger has the following advantages:

- (1) the charge efficiency is high;
- (2) the amount of ozone generated during charging is little;
- (3) the image forming apparatus can be minimized in size;
- (4) the charger is hardly contaminated by the toner used or the like materials; and
- (5) the surface of the photoreceptor is hardly abraded.

In addition, it is preferable for the charger to apply a DC voltage overlapped with an AC voltage to avoid uneven charging.

When such contact chargers and short-range chargers are used, dielectric break down of the photoreceptor tends to occur. However, the photoreceptor of the present invention has good resistance to break down. This is because the photoreceptor has an intermediate layer including the charge blocking layer and the moiré preventing layer, and in addition the photosensitive layer thereof include no coarse particles of charge generation materials. Therefore, the short-range chargers can be used without causing any problems such as the uneven charging problem mentioned above and the dielectric breakdown problem.

Thus the photoreceptor is charged with the charger. In conventional image forming apparatus, the photoreceptors are charged so as to have a relatively low electric field strength (e.g., not higher than 40 V/ $\mu\text{m}$ , preferably not higher than 30 V/ $\mu\text{m}$ ) to avoid background development due to the photoreceptor. Namely, when the electric field strength of a photoreceptor increases, the probability that images produced by the photoreceptor have background development increases. However, when the electric field strength is decreased, the photo-carrier generating efficiency is also decreased, resulting in deterioration of photosensitivity of the photoreceptor. Additionally, in this case the strength of the electric field formed between the surface of the photoreceptor and the electroconductive substrate thereof is decreased, and therefore the photo-carriers generated in the photosensitive layer cannot move straight, and scatter due to coulomb repulsion, resulting in deterioration of resolution of the electrostatic latent images formed on the photoreceptor. When the photoreceptor of the present invention is used, the probability of occurrence of background development can be extremely decreased. Therefore, it is not necessary to decrease the electric field strength more than necessary, and the photoreceptor can be used at an electric field strength not greater than 40 V/ $\mu\text{m}$ . Therefore, photodecaying of the photoreceptor can be well performed under such conditions, and the resultant electrostatic latent images can be well developed with wide margin. Therefore, the electrostatic latent images can be developed without deteriorating the resolution thereof.

Light sources with high intensity such as light emitting diodes (LEDs), laser diodes (LDs) and electroluminescent lamps (EL) can be used for the imagewise light irradiator 15.

Suitable light sources for use in the discharging lamp 12 include fluorescent lamps, tungsten lamps, halogen lamps, mercury lamps, sodium lamps, light emitting diodes (LEDs), laser diodes (LDs), light sources using electroluminescent lamps (EL), and the like. In addition, in order to obtain light having a desired wave length range, filters such as sharp-cut filters, band pass filters, near-infrared cutting filters, dichroic filters, interference filters, color temperature converting filters and the like can be used.

Among these light sources, LEDs, and LDs are preferably used because of emitting a high energy light beam having a wavelength of from 600 nm to 800 nm, to which the titanyl phthalocyanine pigment in the charge generation layer has high sensitivity.

The above-mentioned lamps can be used for not only the processes mentioned above and illustrated in FIG. 12, but also other processes using light irradiation, such as a transfer process including light irradiation, a discharging process, a cleaning process including light irradiation and a pre-exposure process.

Referring to FIG. 12m, when the toner image formed on the photoreceptor 11 by the developing unit 16 is transferred onto the receiving paper 19, all of the toner particles of the toner image are not transferred on the receiving paper 19, and toner particles remain on the surface of the photoreceptor 11. The residual toner particles are removed from the photoreceptor 11 by the fur brush 24 or the cleaning blade 25. The residual toner particles remaining on the photoreceptor 11 can be removed by only a cleaning brush. Suitable cleaning brushes include known cleaning brushes such as fur brushes and mag-fur brushes.

When the photoreceptor 11 which is previously charged positively (or negatively) is exposed to imagewise light, an electrostatic latent image having a positive (or negative) charge is formed on the photoreceptor 11. When the latent image having a positive (or negative) charge is developed with a toner having a negative (or positive) charge, a positive image can be obtained. In contrast, when the latent image having a positive (negative) charge is developed with a toner having a positive (negative) charge, a negative image (i.e., a reversal image) can be obtained. As the developing method, known developing methods can be used. In addition, as the discharging methods, known discharging methods can also be used.

FIG. 14 illustrates another embodiment of the image forming apparatus of the present invention. Numeral 41 designates a photoreceptor which is the photoreceptor of the mentioned above.

Referring to FIG. 14, the photoreceptor 41 has a belt-form. The photoreceptor 41 is rotated by rollers 42a and 42b. The photoreceptor 41 is charged with a charger 43, and then exposed to imagewise light emitted by an imagewise light irradiator 44 to form an electrostatic latent image on the photoreceptor 41. The latent image is developed with a developing device 49 to form a toner image on the photoreceptor 41. The toner image is transferred onto a receiving paper (not shown) using a transfer charger 45. After the toner image transferring process, the surface of the photoreceptor 41 is cleaned with a cleaning brush 47 after performing a pre-cleaning light irradiating operation using a pre-cleaning light irradiator 46. Then the photoreceptor 41 is discharged by being exposed to light emitted by a discharging light source 48. In the pre-cleaning light irradiating process, light irradiates the photoreceptor 41 from the substrate side of the photoreceptor 41. In this case, the substrate has to be light-transmissive.

The image forming apparatus of the present invention is not limited to the image forming apparatus as shown in FIGS. 12-14. For example, in FIG. 14, the pre-cleaning light irradiating operation can be performed from the photosensitive layer side of the photoreceptor 41. In addition, the light irradiation in the light image irradiating process and the discharging process may be performed from the substrate side of the photoreceptor 41.

Further, a pre-transfer light irradiation operation, which is performed before the transferring of the toner image, and a

preliminary light irradiation operation, which is performed before the imagewise light irradiation, and other light irradiation operations may also be performed.

The above-mentioned image forming unit may be fixedly set in an image forming apparatus such as copiers, facsimiles and printers. However, the image forming unit may be set therein as a process cartridge. The process cartridge means an image forming unit which includes a photoreceptor and at least one of a charger, an imagewise light irradiator, an image developer, an image transfer device and a cleaner.

FIG. 15 is a schematic view illustrating an embodiment of the process cartridge of the present invention. In FIG. 15, the process cartridge includes a photoreceptor 51 which is the photoreceptor of the present invention, a charging roller 53 configured to charge the photoreceptor 51, an imagewise light irradiating section 54 configured to irradiate the photoreceptor 51 with imagewise light to form an electrostatic latent image on the photoreceptor 51, an image developer (a developing roller) 55 configured to develop the latent image with a toner, an image transfer device 56 configured to transfer the toner image onto a receiving paper, a cleaning brush 57 configured to clean the surface of the photoreceptor 51, and a housing 58.

Then, a full color image forming apparatus which is an embodiment of the image forming apparatus of the present invention will be explained.

FIG. 16 is a schematic view illustrating another embodiment of the image forming apparatus (a tandem type image forming apparatus) of the present invention, which includes plural image forming units. However, the image forming apparatus of the present invention is not limited thereto.

In FIG. 16, the tandem type image forming apparatus has a cyan image forming unit 66C, a magenta image forming unit 66M, a yellow image forming unit 66Y and a black image forming unit 66K. Drum photoreceptors 61C, 61M, 61Y and 61K, which are the photoreceptor of the present invention, rotate in the direction indicated by the respective arrows. Around the photoreceptors 61C, 61M, 61Y and 61K, chargers 62C, 62M, 62Y and 62K, image developers 64C, 64M, 64Y and 64K, and cleaners 65C, 65M, 65Y and 65K are arranged in this order in the clockwise direction. As the chargers, the above-mentioned chargers which can uniformly charge the surface of the photoreceptors are preferably used. Imagewise light irradiators 63C, 63M, 63Y and 63K irradiate a surface of the respective photoreceptors located between the chargers and the image developers with laser light to form an electrostatic latent image on the respective photoreceptors. The four image forming units 66C, 66M, 66Y and 66K are arranged along a transfer belt 70. The transfer belt 70 contacts the respective photoreceptor 61C, 61M, 61Y or 61K at an image transfer point located between the respective image developer and the respective cleaner to receive color images formed on the photoreceptors. At the backsides of the image transfer points of the transfer belt 70, transfer brushes 71C, 71M, 71Y and 71K are arranged to apply a transfer bias to the transfer belt 70.

The image forming process will be explained referring to FIG. 16.

At first, in each of the image forming units 66C, 66M, 66Y and 66K, the photoreceptor 61C, 61M, 61Y or 61K is charged with the charger 62C, 62M, 62Y or 62K which rotates in the direction indicated by an arrow. Then an image irradiator (not shown) irradiates each of the photoreceptors 61C, 61M, 61Y and 61K with laser light 63C, 63M, 63Y or 63K to form an electrostatic latent image on each photoreceptor.

Then the electrostatic latent image on each photoreceptor is developed with the image developer 64C, 64M, 64Y or 64K including a color toner C, M, Y or K to form a color toner image on each photoreceptor. The thus prepared color toner images are transferred onto a receiving material 67 fed from a paper tray.

The receiving material 67 is fed by a feeding roller 68 and stops at a pair of registration rollers 69, and is timely fed to the transfer belt 70 such that the color toner images formed on each photoreceptor are transferred onto proper positions of the receiving material 67. Each of the toner images on the photoreceptors is transferred onto the receiving material 67 at the contact point (i.e., the transfer position) of the photoreceptor and the receiving material 67.

The toner image on each photoreceptor is transferred onto the receiving material 67 due to an electric field which is formed due to the difference between the transfer bias voltage and the potential of the photoreceptor. After passing through the four transfer positions, the receiving material 67 having the color toner images thereon is then transported to a fixer 72 so that the color toner images are fixed to the receiving material 67. Then the receiving material 67 is discharged from the main body of the image forming apparatus. Toner particles, which remain on the photoreceptors even after the transfer process, are collected by respective cleaners 65C, 65M, 65Y and 65K.

In the image forming apparatus, the image forming units 66C, 66M, 66Y and 66K are arranged in this order in the paper feeding direction, but the order is not limited thereto. In addition, although the color toner images are directly transferred onto a receiving material in this image forming apparatus, the toner images can be transferred to the receiving material via an intermediate transfer medium.

When a black image is formed, the other image forming units 66C, 66M and 66Y may be stopped. In addition, in FIG. 16, the chargers 62C, 62M, 62Y and 62K contact the respective photoreceptors 61C, 61M, 61Y and 61K, but the chargers may be short-range charges in which a proper gap of from 10 to 200  $\mu$ m is formed between the charging members and the respective photoreceptors. Such short-range chargers have advantages such that the abrasion of the photoreceptors and the chargers can be reduced, and in addition a toner film is hardly formed on the charging members.

Having generally described this invention, further understanding can be obtained by reference to certain specific examples which are provided herein for the purpose of illustration only and are not intended to be limiting. In the descriptions in the following examples, the numbers represent weight ratios in parts, unless otherwise specified.

## EXAMPLES

At first, the method of synthesizing the charge generating material for use in the photoreceptor of the present invention is explained.

### Comparative Synthesis Example 1

A titanyl phthalocyanine pigment was prepared by the method described in JP-A 2001-19871. Specifically, in a container 29.2 g of 1,3-diiminoisoindoline and 200 ml of sulforane were mixed while stirring. Under a nitrogen gas flow, 20.4 g of titanium tetrabutoxide were dropped therein. After the addition of titanium tetrabutoxide was completed, the temperature of the mixture was gradually increased to 180° C. The temperature of the mixture was maintained in

a range of from 170° C. to 180° C. for 5 hours while stirring the mixture to react the compounds. After the reaction was terminated, the reaction product was cooled. Then the reaction product was filtered to obtain the precipitate. Then the precipitate was washed with chloroform until the precipitate colored blue. The precipitate was then washed with methanol several times, followed by washing with hot water of 80° C. several times. Thus a crude titanyl phthalocyanine was prepared.

One part of the thus prepared crude titanyl phthalocyanine was gradually added to 20 parts of concentrated sulfuric acid to be dissolved therein. The solution was gradually added to 100 parts of ice water while stirred, to precipitate a titanyl phthalocyanine pigment. The pigment was obtained by filtering. The pigment was washed until the filtrate became neutral. In this case, the pH of the filtrate was 6.8. Forty (40) grams of the thus prepared aqueous wet cake of the titanyl phthalocyanine pigment, which has a solid content of 15% by weight, were added to 200 g of tetrahydrofuran (THF) and the mixture was stirred for about 4 hours. In this case, the ratio of the pigment to the crystal change solvent (THF) was 1:33. Then the mixture was filtered to obtain a titanyl phthalocyanine pigment 1. The pigment was dried to prepare a titanyl phthalocyanine powder. The materials used for the titanyl phthalocyanine pigment does not include a halogenated compound.

When the thus prepared titanyl phthalocyanine pigment 1 was subjected to an X-ray diffraction analysis using a Cu—K  $\alpha$  X-ray having a wavelength of 1.542  $\text{\AA}$ , the powder had an X-ray diffraction spectrum such that a maximum peak is observed at a Bragg (20) angle of 27.2 $\pm$ 0.2°, and a lowest angle peak at an angle of 7.3 $\pm$ 0.2°, wherein no peak is observed between the peaks of 7.3° and 9.4° and at an angle of 26.3. The X-ray diffraction spectrum thereof is illustrated in FIG. 17.

In addition, a part of the aqueous wet cake prepared above was dried at 80° C. for 2 days under a reduced pressure of 5 mmHg, to prepare a titanyl phthalocyanine powder having a low crystallinity. The X-ray diffraction spectrum thereof is illustrated in FIG. 18.

The measuring conditions were as follows:

X-ray tube: Cu  
Voltage: 50 kV  
Current: 30 mA  
Scanning speed: 2°/min  
Scanning range: 3° to 40°  
Time constant: 2 seconds

### Comparative Synthesis Example 2

A titanyl phthalocyanine pigment was prepared using the method described in Example 1 of JP-A 01-299874. Specifically, the procedure for preparation of the wet cake in Comparative Synthesis Example 1 was repeated. The wet cake was dried to prepare the titanyl phthalocyanine pigment. One gram of the titanyl phthalocyanine pigment was mixed with 50 g of polyethylene glycol, and the mixture was milled using 100 g of glass beads to change the crystal form. Then the titanyl phthalocyanine pigment was washed with diluted sulfuric acid, followed by washing with ammonium hydroxide and drying. Thus a titanyl phthalocyanine pigment 2 was prepared. The raw materials used for the titanyl phthalocyanine pigment 2 does not include a halogenated compound.

39

## Comparative Synthesis Example 3

A titanyl phthalocyanine pigment was prepared using the method described in Example 1 of JP-A 03-269064. Specifically, the procedure for preparation of the wet cake in Comparative Synthesis Example 1 was repeated. The wet cake was dried to prepare the titanyl phthalocyanine pigment. One gram of the titanyl phthalocyanine pigment was mixed with 10 g of ion-exchange water and 1 g of monochlorobenzene, and the mixture was agitated for one hour at 50° C., to change the crystal form. Then the titanyl phthalocyanine pigment was washed with methanol, followed by washing with ion-exchange water and drying. Thus a titanyl phthalocyanine pigment 3 was prepared. The raw materials used for the titanyl phthalocyanine pigment 3 does not include a halogenated compound.

## Comparative Synthesis Example 4

A titanyl phthalocyanine pigment was prepared using the method described in Example 1 of JP-A 02-8256. Specifically, in a container 982 g of phthalodinitrile and 75 ml of 1-chloronaphthalene were mixed while stirring. Under a nitrogen gas flow, 2.2 ml of titanium tetrachloride were dropped therein. After the addition of titanium tetrachloride was completed, the temperature of the mixture was gradually increased to 200° C. The temperature of the mixture was maintained in a range of from 200° C. to 220° C. for 3 hours while stirring the mixture to react the compounds. After the reaction was terminated, the reaction product was cooled to 130° C. Then the reaction product was filtered to obtain the precipitate. Then the precipitate was washed with 1-chloronaphthalene until the precipitate colored blue. The precipitate was then washed with methanol several times, followed by washing with hot water of 80° C. several times and drying. Thus a titanyl phthalocyanine pigment 4 was prepared. The raw materials used for the titanyl phthalocyanine pigment 4 include a halogenated compound.

## Comparative Synthesis Example 5

A titanyl phthalocyanine pigment was prepared using the method described in Example 1 of JP-A 64-17066. Specifically, 5 parts of a form titanyl phthalocyanine, 10 g of sodium chloride and 5 g of acetophenone were milled for 10 hours at 100° C. using a sand grinder to change the crystal form of the titanyl phthalocyanine. Then the titanyl phthalocyanine pigment was washed with deionized water, followed by washing with methanol and refining with diluted sulfuric acid. Then the pigment was washed with ion-exchange water to an extent such that the filtrate includes no acidic component, followed by drying. Thus a titanyl phthalocyanine pigment 5 was prepared. The raw materials used for the titanyl phthalocyanine pigment 5 include a halogenated compound.

## Comparative Synthesis Example 6

A titanyl phthalocyanine pigment was prepared using the method described in Example 1 of JP-A 11-5919. Specifically, in a container containing 50 g of quinoline, 20.4 g of o-phthalodinitrile and 7.6 g of titanium tetrachloride were reacted at 200° C. for 2 hours. After the reaction, the solvent was removed by a steam distillation. Then the reaction product was refined with a 2% aqueous solution of hydrochloric acid, followed by refinement using a 2% sodium hydroxide. Then the precipitate was washed with methanol,

40

followed by washing with N,N-dimethylformamide and drying. Thus a titanyl phthalocyanine pigment was prepared. Two grams of the titanyl phthalocyanine were gradually dissolved in 40 g of 98% sulfuric acid with a temperature of 5° C. The mixture was agitated for 1 hour at 5° C. Then the solution was gradually added to 400 g of ice water while agitating to precipitate a crystal. The resultant crystal was filtered, followed by washing with distilled water to an extent such that the acid does not remain in the filtrate. Thus, a wet cake was prepared. The wet cake was mixed with 100 g of tetrahydrofuran and the mixture was agitated for 5 hours. Then the mixture was filtered, followed by washing with tetrahydrofuran and drying. Thus, a titanyl phthalocyanine pigment 6 was prepared. The raw materials used for the titanyl phthalocyanine pigment 6 include a halogenated compound.

## Comparative Synthesis Example 7

A titanyl phthalocyanine pigment was prepared using the method described in Example 1 of JP-A 03-255456. Specifically, the procedure for preparation of the wet cake in Comparative Synthesis Example 1 was repeated. Ten (10) grams of the wet cake were mixed with 15 g of sodium chloride and 7 g of diethylene glycol and the mixture was milled for 60 hours at 80° C. using an automatic mortar. Then the pigment was washed with water to remove sodium chloride and diethylene glycol therefrom. The dispersion was dried under a reduced pressure to prepare a powder. The powder was mixed with 200 g of cyclohexanone and the mixture was subjected to sand milling for 30 minutes using glass beads with a diameter of 1 mm. Thus, a titanyl phthalocyanine pigment 7 was prepared. The raw materials used for the titanyl phthalocyanine pigment 7 does not include a halogenated compound.

## Comparative Synthesis Example 8

A titanyl phthalocyanine pigment was prepared using the method described in Example 1 of JP-A 08-110649. Specifically, 58 g of 1,3-diiminoisoindoline and 51 g of tetrabuthoxy titanium were reacted in 300 ml of  $\alpha$ -chloronaphthalene for 5 hours at 210° C. Then the reaction product was washed with  $\alpha$ -chloronaphthalene, followed by washing with dimethylformamide. Then the reaction product was washed with hot dimethylformamide, followed by washing with hot water. Further, the reaction product was washed with methanol, followed by drying. Thus, 50 g of a titanyl phthalocyanine was prepared. Four (4) grams of the titanyl phthalocyanine were added to 400 g of concentrated sulfuric acid cooled to 0° C., and the mixture was agitated for 1 hour at 0° C. After the titanyl phthalocyanine was perfectly dissolved, the solution was added to a mixture of 800 ml of water and 800 ml of toluene which had been cooled to 0° C. After being mixed for 2 hours at room temperature, the precipitated phthalocyanine crystal was filtered. The cake was washed with methanol, followed by washing with water and filtering. After the filtrate became neutral, the phthalocyanine crystal was filtered, followed by drying. Thus, 2.9 g of a titanyl phthalocyanine pigment 8 were prepared. The raw materials used for the titanyl phthalocyanine pigment 8 does not include a halogenated compound.

## Synthesis Example 1

The procedure for preparation of the aqueous wet cake in Comparative Synthesis Example 1 was repeated. Then the

pigment was subjected to the crystal change treatment mentioned below, to prepare a titanyl phthalocyanine crystal having a primary particle diameter smaller than that of the crystal prepared in Comparative Synthesis Example 1.

Specifically, 60 g of the aqueous wet paste, which had not been subjected to a crystal change treatment and which has a solid content of 15% by weight, was mixed with 400 g of tetrahydrofuran (THF) and the mixture was strongly agitated at room temperature using a homomixer MARK II model manufactured by Kenis Ltd., whose rotor was rotated at a revolution of 2,000 rpm. In this case, the ratio of the pigment to the crystal change solvent (THF) was 1:44. When the color of the paste was changed from dark blue to light blue (20 minutes after the start of agitation), the agitation was stopped, and the dispersion was filtered under a reduced pressure. The thus prepared crystal on the filtering device was washed with tetrahydrofuran. Thus, a wet cake of a pigment. The wet cake was dried for 2 days at 70° C. under a reduced pressure of 5 mmHg. Thus, 8.5 g of a titanyl phthalocyanine pigment 9 were prepared. The raw materials used for the titanyl phthalocyanine pigment 9 does not include a halogenated compound.

A part of the aqueous wet paste of the titanyl phthalocyanine prepared in Comparative Example 1, which had not been subjected to a crystal change treatment, was diluted with ion-exchange water such that the resultant dispersion has a solid content of 1% by weight. The titanyl phthalocyanine was placed on a 150-mesh copper covered with a continuous collodion membrane and a conductive carbon layer. The titanyl phthalocyanine was observed with a transmission electron microscope (H-9000NAR from Hitachi Ltd., hereinafter referred to as a TEM) of 75,000 power magnification to measure the average particle size of the titanyl phthalocyanine prepared in Comparative Synthesis Example 1. The average particle diameter thereof was determined as follows.

The images of particles of the titanyl phthalocyanine in the TEM were photographed. Among the particles (needle form particles) of the titanyl phthalocyanine in the photograph, 30 particles were randomly selected to measure the lengths of the particles in the long axis direction. The lengths were arithmetically averaged to determine the average particle diameter of the titanyl phthalocyanine.

As a result, the titanyl phthalocyanine in the aqueous wet paste prepared in Comparative Synthesis Example 1 has an average primary particle diameter of about 0.06  $\mu\text{m}$ .

Similarly, each of the titanyl phthalocyanine crystals prepared in Comparative Synthesis Example 1 and Synthesis Example 1, which had been subjected to the crystal change treatment but was not filtered, was diluted with tetrahydrofuran such that the resultant dispersion has a solid content of 1% by weight. The average particle diameters of the titanyl phthalocyanine crystals were determined by the method mentioned above. The results are shown in Table 1. In this regard, the form of the crystals was not uniform and includes triangle forms, quadrangular forms, etc. Therefore, the maximum lengths of the diagonal lines of the particles were arithmetically averaged.

It is clear from Table 1 that the pigment 1 prepared in Comparative Synthesis Example 1 has a large average particle diameter and in addition includes coarse particles. In contrast, the pigment 9 prepared in Synthesis Example 1 has a small average particle diameter and the particle size of the particles is uniform.

TABLE 1

| Pigment                            | Average particle diameter ( $\mu\text{m}$ ) | Note                                                                                       |
|------------------------------------|---------------------------------------------|--------------------------------------------------------------------------------------------|
| Pigment 1<br>(Comp. Syn.<br>Ex. 1) | 0.31                                        | Coarse particles having a particle diameter of from 0.3 to 0.4 $\mu\text{m}$ are included. |
| Pigment 9<br>(Syn. Ex. 1)          | 0.12                                        | The particle diameters of the crystal are almost uniform.                                  |

It was confirmed that the X-ray diffraction spectra of the pigments prepared in Comparative Synthesis Examples 2 to 8 are the same as those described in the respective patent publications. The X-ray spectrum of the pigment 9 prepared in Synthesis Example 1 is the same as that of the pigment 1 prepared in Comparative Synthesis Example 1. The peaks of the X-ray spectra of the pigments 1-9 are described in Table 2.

TABLE 2

| Pigment<br>No. | Max.<br>Peak | angle<br>peak | Lowest       |              |             | peak<br>between<br>7.3°<br>and<br>9.4° |  |  | 24.0°<br>peak | 26.3°<br>peak |
|----------------|--------------|---------------|--------------|--------------|-------------|----------------------------------------|--|--|---------------|---------------|
|                |              |               | 9.4°<br>peak | 9.6°<br>peak | and<br>9.4° |                                        |  |  |               |               |
| 1              | 27.2°        | 7.3°          | Yes          | Yes          | No          | Yes                                    |  |  | No            |               |
| 2              | 27.2°        | 7.3°          | No           | No           | No          | Yes                                    |  |  | No            |               |
| 3              | 27.2°        | 9.6°          | Yes          | Yes          | No          | Yes                                    |  |  | No            |               |
| 4              | 27.2°        | 7.4°          | No           | Yes          | No          | No                                     |  |  | No            |               |
| 5              | 27.2°        | 7.3°          | Yes          | Yes          | Yes         | Yes                                    |  |  | No            |               |
| 6              | 27.2°        | 7.5°          | No           | Yes          | Yes         | Yes                                    |  |  | No            |               |
| 7              | 27.2°        | 7.4°          | No           | No           | Yes         | Yes                                    |  |  | Yes           |               |
| 8              | 27.2°        | 7.3°          | Yes          | Yes          | No          | Yes                                    |  |  | No            |               |
| 9              | 27.2°        | 7.3°          | Yes          | Yes          | No          | Yes                                    |  |  | No            |               |

## Dispersion Preparation Example 1

A dispersion having the following formula was prepared using the titanyl phthalocyanine pigment 1 prepared in Comparative Synthesis Example 1.

|                                                                      |           |
|----------------------------------------------------------------------|-----------|
| Titanyl phthalocyanine pigment 1                                     | 15 parts  |
| Polyvinyl butyral<br>(S-LFC BX-1 from Sekisui<br>Chemical Co., Ltd.) | 10 parts  |
| 2-butanone                                                           | 280 parts |

At first, the polyvinyl butyral resin was dissolved in 2-butanone. Then titanyl phthalocyanine pigment 1 was dispersed for 30 minutes in the resin solution using a dispersion machine including PSZ balls with a particle diameter of 0.5 mm while the rotor was rotated at a revolution of 1200 rpm. Thus, a dispersion 1 was prepared.

## Dispersion Preparation Examples 2-9

The procedure for preparation of the dispersion 1 in Dispersion Preparation Example 1 was repeated except that titanyl phthalocyanine pigment 1 was replaced with titanyl phthalocyanine pigments 2-9. Thus, dispersions 2-9 were prepared.

## Dispersion Preparation Example 10

The dispersion 1 prepared in Dispersion Preparation Example 1 was subjected to filtering using a cotton wind cartridge filter TCW-1-CS with an effective pore diameter of 1  $\mu\text{m}$ , which is manufactured by ADVANTECH, while applying a pressure using a pump. Thus, a dispersion 10 was prepared.

## Dispersion Preparation Example 11

The procedure for preparation of the dispersion 10 in Dispersion Preparation Example 10 was repeated except that the filter was replaced with a cotton wind cartridge filter TCW-3-CS with an effective pore diameter of 3  $\mu\text{m}$ , which is manufactured by ADVANTECH. Thus, a dispersion 11 was prepared.

## Dispersion Preparation Example 12

The procedure for preparation of the dispersion 10 in Dispersion Preparation Example 10 was repeated except that the filter was replaced with a cotton wind cartridge filter TCW-5-CS with an effective pore diameter of 5  $\mu\text{m}$ , which is manufactured by ADVANTECH. Thus, a dispersion 12 was prepared.

## Dispersion Preparation Example 13

The procedure for preparation of the dispersion 1 in Dispersion Preparation Example 1 was repeated except that the rotor was rotated for 20 minutes at a revolution of 1,000 rpm. Thus, a dispersion 13 was prepared.

## Dispersion Preparation Example 14

The dispersion 13 prepared in Dispersion Preparation Example 13 was subjected to filtering using a cotton wind cartridge filter TCW-1-CS with an effective pore diameter of 1  $\mu\text{m}$ , which is manufactured by ADVANTECH, while applying a pressure using a pump. However, the filter was clogged with coarse particles of the dispersion 13, and therefore all the dispersion could not be filtered. Therefore, the dispersion could not be evaluated.

The particle diameter distributions of the pigment particles in the thus prepared dispersions 1-13 were determined using an instrument CAPA 700 from Horiba Ltd.

The results are shown in Table 3.

TABLE 3

| Dispersion | Average particle diameter ( $\mu\text{m}$ ) | Standard Deviation ( $\mu\text{m}$ ) |
|------------|---------------------------------------------|--------------------------------------|
| 1          | 0.29                                        | 0.18                                 |
| 2          | 0.28                                        | 0.19                                 |
| 3          | 0.31                                        | 0.20                                 |
| 4          | 0.30                                        | 0.20                                 |
| 5          | 0.27                                        | 0.19                                 |
| 6          | 0.29                                        | 0.20                                 |
| 7          | 0.27                                        | 0.18                                 |
| 8          | 0.26                                        | 0.19                                 |
| 9          | 0.19                                        | 0.13                                 |
| 10         | 0.22                                        | 0.16                                 |
| 11         | 0.24                                        | 0.17                                 |
| 12         | 0.28                                        | 0.18                                 |
| 13         | 0.33                                        | 0.23                                 |

## Comparative Example 1

## Preparation of Charge Blocking Layer

The following components were mixed to prepare a charge blocking layer coating liquid.

|    |                                                       |          |
|----|-------------------------------------------------------|----------|
| 10 | Alcohol-soluble nylon (AMILAN CM8000 from Toray Ltd.) | 4 parts  |
|    | Methanol                                              | 70 parts |
|    | n-butanol                                             | 30 parts |

The thus prepared CGL coating liquid was coated on an aluminum drum (specified in JIS1050), which has an outside diameter of 60 mm, and the coated liquid was dried to form a charge blocking layer having a thickness of 0.5  $\mu\text{m}$ .

## Preparation of Moiré Preventing Layer

The following components were mixed to prepare a moiré preventing layer coating liquid.

|    |                                                                                                           |            |
|----|-----------------------------------------------------------------------------------------------------------|------------|
| 25 | Titanium oxide (CR-EL from Ishihara Sangyo Kaisha Ltd., average particle diameter of 0.25 $\mu\text{m}$ ) | 84 parts   |
|    | Alkyd resin (BEKKOLITE M6401-50-S from Dainippon Ink & Chemicals, Inc., solid content of 50%)             | 33.6 parts |
|    | Melamine resin (SUPER BEKKAMIN L-121-60 from Dainippon Ink & Chemicals, Inc., solid content of 60%)       | 18.7 parts |
|    | 2-butanone                                                                                                | 100 parts  |

The thus prepared moiré preventing layer coating liquid was coated on the charge blocking layer, and the coated liquid was dried to form a moiré preventing layer having a thickness of 3.5  $\mu\text{m}$ .

In this case, the volume ratio of the inorganic pigment (titanium oxide) to the binder resin is 1/1. The weight ratio of the alkyd resin to the melamine resin is 6/4.

## Preparation of Charge Generation Layer

Dispersion 1 prepared above was coated on the moiré preventing layer, and the coated liquid was dried to form a charge generation layer. The thickness of the charge generation layer was adjusted such that the charge generation layer has a transmittance of 20% against light with a wavelength of 780 nm. In this regard, the transmittance was determined as follows:

- (1) the charge generation layer coating liquid is coated on a polyethylene terephthalate film wound on an aluminum cylinder which is the same as the aluminum cylinder mentioned above;
- (2) the coated liquid is dried to form a charge generation layer on the polyethylene terephthalate film; and
- (3) the transmittance of the film bearing the charge generation layer against light with a wavelength of 780 nm is measured with a spectrophotometer (UV-3100 from Shimadzu Corp.) while compared with the transmittance of the film bearing no charge generation layer thereon.

## 45

## Preparation of Charge Transport Layer

The following components were mixed to prepare a CTL coating liquid.

|                                                                                       |          |
|---------------------------------------------------------------------------------------|----------|
| Polycarbonate (TS2050 from Teijin Chemicals Ltd.)<br>CTM having the following formula | 10 parts |
|                                                                                       | 7 parts  |
|                                                                                       |          |
| Methylene chloride                                                                    | 80 parts |

The thus prepared charge transport layer coating liquid was coated on the charge generation layer and then dried. Thus a charge transport layer having a thickness of 23  $\mu\text{m}$  was prepared.

Thus, a photoreceptor of Example 1 was prepared.

## Comparative Examples 2-10 and Examples 1-3

The procedure for preparation of the photoreceptor in Comparative Example 1 was repeated except that dispersion 1 used for forming the charge generation layer was replaced with dispersions 2-13. Thus, photoreceptors of Comparative Examples 2-10 and Examples 1-3 were prepared. The numbers of the dispersions used in Comparative Examples 2-10 and Examples 1-3 are described in Table 4.

## Comparative Example 11

The procedure for preparation of the photoreceptor in Example 1 was repeated except that the charge blocking layer was not formed. Thus, a photoreceptor of Comparative Example 11 was prepared.

## Comparative Example 12

The procedure for preparation of the photoreceptor in Example 1 was repeated except that the moiré preventing layer was not formed. Thus, a photoreceptor of Comparative Example 12 was prepared.

## Comparative Example 13

The procedure for preparation of the photoreceptor in Example 1 was repeated except that the location of the charge blocking layer and the moiré preventing layer was reversed (i.e., the charge blocking layer was formed on the moiré preventing layer formed on the substrate). Thus, a photoreceptor of Comparative Example 13 was prepared.

## Example 4

The procedure for preparation of the photoreceptor in Example 1 was repeated except that the thickness of the

## 46

charge blocking layer was changed to 0.3  $\mu\text{m}$ . Thus, a photoreceptor of Example 4 was prepared.

## Example 5

The procedure for preparation of the photoreceptor in Example 1 was repeated except that the thickness of the charge blocking layer was changed to 1.0  $\mu\text{m}$ . Thus, a photoreceptor of Example 5 was prepared.

## Example 6

The procedure for preparation of the photoreceptor in Example 1 was repeated except that the thickness of the charge blocking layer was changed to 2.0  $\mu\text{m}$ . Thus, a photoreceptor of Example 6 was prepared.

## Example 7

The procedure for preparation of the photoreceptor in Example 1 was repeated except that the thickness of the charge blocking layer was changed to 0.1  $\mu\text{m}$ . Thus, a photoreceptor of Example 7 was prepared.

## Example 8

The procedure for preparation of the photoreceptor in Example 1 was repeated except that the formula of the moiré preventing layer coating liquid was changed as follows.

| Formula of moiré preventing layer coating liquid                                                             |            |
|--------------------------------------------------------------------------------------------------------------|------------|
| Titanium oxide<br>(CR-EL from Ishihara Sangyo Kaisha Ltd., average particle diameter of 0.25 $\mu\text{m}$ ) | 252 parts  |
| Alkyd resin<br>(BEKKOLITE M6401-50-S from Dainippon Ink & Chemicals, Inc., solid content of 50%)             | 33.6 parts |
| Melamine resin<br>(SUPER BEKKAMIN L-121-60 from Dainippon Ink & Chemicals, Inc., solid content of 60%)       | 18.7 parts |
| 2-butanone                                                                                                   | 300 parts  |

In this case, the volume ratio of the inorganic pigment (titanium oxide) to the binder resin is 3/1. The weight ratio of the alkyd resin to the melamine resin is 6/4.

## Example 9

The procedure for preparation of the photoreceptor in Example 1 was repeated except that the formula of the moiré preventing layer coating liquid was changed as follows.

| Formula of moiré preventing layer coating liquid                                                             |            |
|--------------------------------------------------------------------------------------------------------------|------------|
| Titanium oxide<br>(CR-EL from Ishihara Sangyo Kaisha Ltd., average particle diameter of 0.25 $\mu\text{m}$ ) | 58.8 parts |

-continued

| Formula of moiré preventing layer coating liquid                                                             |            |
|--------------------------------------------------------------------------------------------------------------|------------|
| Alkyd resin<br>(BEKKOLITE M6401-50-S<br>from Dainippon Ink &<br>Chemicals, Inc.,<br>solid content of 50%)    | 33.6 parts |
| Melamine resin<br>(SUPER BEKKAMIN L-121-60<br>from Dainippon Ink & Chemicals,<br>Inc., solid content of 60%) | 18.7 parts |
| 2-butanone                                                                                                   | 150 parts  |

In this case, the volume ratio of the inorganic pigment (titanium oxide) to the binder resin is 0.7/1. The weight ratio of the alkyd resin to the melamine resin is 6/4.

## Example 10

The procedure for preparation of the photoreceptor in Example 1 was repeated except that the formula of the moiré preventing layer coating liquid was changed as follows.

| Formula of moiré preventing layer coating liquid                                                               |            |
|----------------------------------------------------------------------------------------------------------------|------------|
| Titanium oxide<br>(CR-EL from Ishihara<br>Sangyo Kaisha Ltd.,<br>average particle<br>diameter of 0.25 $\mu$ m) | 336 parts  |
| Alkyd resin<br>(BEKKOLITE M6401-50-S<br>from Dainippon Ink &<br>Chemicals, Inc.,<br>solid content of 50%)      | 33.6 parts |
| Melamine resin<br>(SUPER BEKKAMIN L-121-60<br>from Dainippon Ink & Chemicals,<br>Inc., solid content of 60%)   | 18.7 parts |
| 2-butanone                                                                                                     | 350 parts  |

In this case, the volume ratio of the inorganic pigment (titanium oxide) to the binder resin is 4/1. The weight ratio of the alkyd resin to the melamine resin is 6/4.

## Example 11

The procedure for preparation of the photoreceptor in Example 1 was repeated except that the formula of the charge blocking layer coating liquid was changed as follows.

| Formula of charge blocking layer coating liquid                                                              |            |
|--------------------------------------------------------------------------------------------------------------|------------|
| Alkyd resin<br>(BEKKOLITE M6401-50-S<br>from Dainippon Ink &<br>Chemicals, Inc.,<br>solid content of 50%)    | 33.6 parts |
| Melamine resin<br>(SUPER BEKKAMIN L-121-60<br>from Dainippon Ink & Chemicals,<br>Inc., solid content of 60%) | 18.7 parts |
| 2-butanone                                                                                                   | 500 parts  |

## Example 12

The procedure for preparation of the photoreceptor in Example 1 was repeated except that the formula of the moiré preventing layer coating liquid was changed as follows.

| Formula of moiré preventing layer coating liquid                                                             |            |
|--------------------------------------------------------------------------------------------------------------|------------|
| Zinc oxide<br>(SAZEX 4000 from<br>Sakai Chemical<br>Industry Co., Ltd.)                                      | 110 parts  |
| Alkyd resin<br>(BEKKOLITE M6401-50-S<br>from Dainippon Ink &<br>Chemicals, Inc.,<br>solid content of 50%)    | 33.6 parts |
| Melamine resin<br>(SUPER BEKKAMIN L-121-60<br>from Dainippon Ink & Chemicals,<br>Inc., solid content of 60%) | 18.7 parts |
| 2-butanone                                                                                                   | 120 parts  |

In this case, the volume ratio of the inorganic pigment (zinc oxide) to the binder resin is 1/1. The weight ratio of the alkyd resin to the melamine resin is 6/4.

## Example 13

The procedure for preparation of the photoreceptor in Example 1 was repeated except that the formula of the moiré preventing layer coating liquid was changed as follows.

| Formula of moiré preventing layer coating liquid                                                               |            |
|----------------------------------------------------------------------------------------------------------------|------------|
| Titanium oxide<br>(CR-EL from Ishihara<br>Sangyo Kaisha Ltd.,<br>average particle<br>diameter of 0.25 $\mu$ m) | 84 parts   |
| Alkyd resin<br>(BEKKOLITE M6401-50-S<br>from Dainippon Ink &<br>Chemicals, Inc.,<br>solid content of 50%)      | 22.4 parts |
| Melamine resin<br>(SUPER BEKKAMIN L-121-60<br>from Dainippon Ink & Chemicals,<br>Inc., solid content of 60%)   | 28 parts   |
| 2-butanone                                                                                                     | 100 parts  |

In this case, the volume ratio of the inorganic pigment (titanium oxide) to the binder resin is 1/1. The weight ratio of the alkyd resin to the melamine resin is 4/6.

## Example 14

The procedure for preparation of the photoreceptor in Example 1 was repeated except that the formula of the moiré preventing layer coating liquid was changed as follows.

| Formula of moiré preventing layer coating liquid              |          |
|---------------------------------------------------------------|----------|
| Titanium oxide<br>(CR-EL from Ishihara<br>Sangyo Kaisha Ltd., | 84 parts |

-continued

| Formula of moiré preventing layer coating liquid                                                          |            |  |
|-----------------------------------------------------------------------------------------------------------|------------|--|
| average particle diameter of 0.25 $\mu\text{m}$ )                                                         |            |  |
| Alkyd resin<br>(BEKKOLITE M6401-50-S<br>from Dainippon Ink & Chemicals, Inc., solid content of 50%)       | 28 parts   |  |
| Melamine resin<br>(SUPER BEKKAMIN L-121-60<br>from Dainippon Ink & Chemicals, Inc., solid content of 60%) | 23.3 parts |  |
| 2-butanone                                                                                                | 100 parts  |  |

In this case, the volume ratio of the inorganic pigment (titanium oxide) to the binder resin is 1/1. The weight ratio of the alkyd resin to the melamine resin is 5/5.

## Example 15

The procedure for preparation of the photoreceptor in Example 1 was repeated except that the formula of the moiré preventing layer coating liquid was changed as follows.

| Formula of moiré preventing layer coating liquid                                                             |            |  |
|--------------------------------------------------------------------------------------------------------------|------------|--|
| Titanium oxide<br>(CR-EL from Ishihara Sangyo Kaisha Ltd., average particle diameter of 0.25 $\mu\text{m}$ ) | 84 parts   |  |
| Alkyd resin<br>(BEKKOLITE M6401-50-S<br>from Dainippon Ink & Chemicals, Inc., solid content of 50%)          | 39.2 parts |  |
| Melamine resin<br>(SUPER BEKKAMIN L-121-60<br>from Dainippon Ink & Chemicals, Inc., solid content of 60%)    | 14 parts   |  |
| 2-butanone                                                                                                   | 100 parts  |  |

In this case, the volume ratio of the inorganic pigment (titanium oxide) to the binder resin is 1/1. The weight ratio of the alkyd resin to the melamine resin is 7/3.

## Example 16

The procedure for preparation of the photoreceptor in Example 1 was repeated except that the formula of the moiré preventing layer coating liquid was changed as follows.

| Formula of moiré preventing layer coating liquid                                                             |            |  |
|--------------------------------------------------------------------------------------------------------------|------------|--|
| Titanium oxide<br>(CR-EL from Ishihara Sangyo Kaisha Ltd., average particle diameter of 0.25 $\mu\text{m}$ ) | 84 parts   |  |
| Alkyd resin<br>(BEKKOLITE M6401-50-S<br>from Dainippon Ink & Chemicals, Inc., solid content of 50%)          | 44.8 parts |  |

-continued

| Formula of moiré preventing layer coating liquid                                                          |           |  |
|-----------------------------------------------------------------------------------------------------------|-----------|--|
| Melamine resin<br>(SUPER BEKKAMIN L-121-60<br>from Dainippon Ink & Chemicals, Inc., solid content of 60%) | 9.3 parts |  |
| 2-butanone                                                                                                | 100 parts |  |

In this case, the volume ratio of the inorganic pigment (titanium oxide) to the binder resin is 1/1. The weight ratio of the alkyd resin to the melamine resin is 8/2.

## Example 17

The procedure for preparation of the photoreceptor in Example 1 was repeated except that the formula of the moiré preventing layer coating liquid was changed as follows.

| Formula of moiré preventing layer coating liquid                                                             |            |  |
|--------------------------------------------------------------------------------------------------------------|------------|--|
| Titanium oxide<br>(CR-EL from Ishihara Sangyo Kaisha Ltd., average particle diameter of 0.25 $\mu\text{m}$ ) | 84 parts   |  |
| Alkyd resin<br>(BEKKOLITE M6401-50-S<br>from Dainippon Ink & Chemicals, Inc., solid content of 50%)          | 50.4 parts |  |
| Melamine resin<br>(SUPER BEKKAMIN L-121-60<br>from Dainippon Ink & Chemicals, Inc., solid content of 60%)    | 4.7 parts  |  |
| 2-butanone                                                                                                   | 100 parts  |  |

In this case, the volume ratio of the inorganic pigment (titanium oxide) to the binder resin is 1/1. The weight ratio of the alkyd resin to the melamine resin is 9/1.

## Example 18

The procedure for preparation of the photoreceptor in Example 1 was repeated except that the formula of the moiré preventing layer coating liquid was changed as follows.

| Formula of moiré preventing layer coating liquid                                                             |           |  |
|--------------------------------------------------------------------------------------------------------------|-----------|--|
| Titanium oxide<br>(CR-EL from Ishihara Sangyo Kaisha Ltd., average particle diameter of 0.25 $\mu\text{m}$ ) | 84 parts  |  |
| Alcohol-soluble nylon<br>(AMILAN CM800<br>from Toray Ltd.)                                                   | 24 parts  |  |
| Methanol                                                                                                     | 300 parts |  |
| 2-butanone                                                                                                   | 130 parts |  |

In this case, the volume ratio of the inorganic pigment (titanium oxide) to the binder resin is 1/1.

**51**

## Example 19

The procedure for preparation of the photoreceptor in Example 1 was repeated except that the formula of the moiré preventing layer coating liquid was changed as follows.

| Formula of moiré preventing layer coating liquid                                                                        |            |
|-------------------------------------------------------------------------------------------------------------------------|------------|
| Titanium oxide<br>(CR-EL from Ishihara<br>Sangyo Kaisha Ltd.,<br>average particle<br>diameter of 0.25 $\mu\text{m}$ )   | 42 parts   |
| Titanium oxide<br>(PT-401M from Ishihara<br>Sangyo Kaisha Ltd.,<br>average particle<br>diameter of 0.07 $\mu\text{m}$ ) | 42 parts   |
| Alkyd resin<br>(BEKKOLITE M6401-50-S<br>from Dainippon Ink &<br>Chemicals, Inc.,<br>solid content of 50%)               | 33.6 parts |
| Melamine resin<br>(SUPER BEKKAMIN L-121-60<br>from Dainippon<br>Ink & Chemicals,<br>Inc., solid content of 60%)         | 18.7 parts |
| 2-butanone                                                                                                              | 100 parts  |

In this case, the volume ratio of the inorganic pigment (titanium oxide) to the binder resin is 1/1, and the weight ratio of the alkyd resin to the melamine resin is 6/4. The ratio of the particle diameter of the smaller titanium oxide (PT-401M) to the larger titanium oxide (CR-EL) is 0.28 and the mixing ratio thereof is 1/1.

## Example 20

The procedure for preparation of the photoreceptor in Example 1 was repeated except that the formula of the moiré preventing layer coating liquid was changed as follows.

| Formula of moiré preventing layer coating liquid                                                                        |            |
|-------------------------------------------------------------------------------------------------------------------------|------------|
| Titanium oxide<br>(CR-EL from Ishihara<br>Sangyo Kaisha Ltd.,<br>average particle<br>diameter of 0.25 $\mu\text{m}$ )   | 75.6 parts |
| Titanium oxide<br>(PT-401M from Ishihara<br>Sangyo Kaisha Ltd.,<br>average particle<br>diameter of 0.07 $\mu\text{m}$ ) | 8.4 parts  |
| Alkyd resin<br>(BEKKOLITE M6401-50-S<br>from Dainippon Ink &<br>Chemicals, Inc.,<br>solid content of 50%)               | 33.6 parts |
| Melamine resin<br>(SUPER BEKKAMIN L-121-60<br>from Dainippon Ink &<br>Chemicals, Inc.,<br>solid content of 60%)         | 18.7 parts |
| 2-butanone                                                                                                              | 100 parts  |

In this case, the volume ratio of the inorganic pigment (titanium oxide) to the binder resin is 1/1, and the weight ratio of the alkyd resin to the melamine resin is 6/4. The ratio

**52**

of the particle diameter of the smaller titanium oxide (PT-401M) to the larger titanium oxide (CR-EL) is 0.28 and the mixing ratio thereof is 9/1.

## Example 21

The procedure for preparation of the photoreceptor in Example 1 was repeated except that the formula of the moiré preventing layer coating liquid was changed as follows.

| Formula of moiré preventing layer coating liquid                                                                        |            |
|-------------------------------------------------------------------------------------------------------------------------|------------|
| Titanium oxide<br>(CR-EL from Ishihara<br>Sangyo Kaisha Ltd.,<br>average particle<br>diameter of 0.25 $\mu\text{m}$ )   | 8.4 parts  |
| Titanium oxide<br>(PT-401M from Ishihara<br>Sangyo Kaisha Ltd.,<br>average particle<br>diameter of 0.07 $\mu\text{m}$ ) | 75.6 parts |
| Alkyd resin<br>(BEKKOLITE M6401-50-S<br>from Dainippon Ink &<br>Chemicals, Inc.,<br>solid content of 50%)               | 33.6 parts |
| Melamine resin<br>(SUPER BEKKAMIN L-121-60<br>from Dainippon Ink &<br>Chemicals, Inc.,<br>solid content of 60%)         | 18.7 parts |
| 2-butanone                                                                                                              | 100 parts  |

In this case, the volume ratio of the inorganic pigment (titanium oxide) to the binder resin is 1/1, and the weight ratio of the alkyd resin to the melamine resin is 6/4. The ratio of the particle diameter of the smaller titanium oxide (PT-401M) to the larger titanium oxide (CR-EL) is 0.28 and the mixing ratio thereof is 1/9.

## Example 22

The procedure for preparation of the photoreceptor in Example 1 was repeated except that the formula of the moiré preventing layer coating liquid was changed as follows.

| Formula of moiré preventing layer coating liquid                                                                       |            |
|------------------------------------------------------------------------------------------------------------------------|------------|
| Titanium oxide<br>(CR-EL from Ishihara<br>Sangyo Kaisha Ltd.,<br>average particle<br>diameter of 0.25 $\mu\text{m}$ )  | 42 parts   |
| Titanium oxide<br>(TTO-F1 from Ishihara<br>Sangyo Kaisha Ltd.,<br>average particle<br>diameter of 0.04 $\mu\text{m}$ ) | 42 parts   |
| Alkyd resin<br>(BEKKOLITE M6401-50-S<br>from Dainippon Ink &<br>Chemicals, Inc.,<br>solid content of 50%)              | 33.6 parts |
| Melamine resin<br>(SUPER BEKKAMIN L-121-60<br>from Dainippon Ink &<br>Chemicals, Inc.,<br>solid content of 60%)        | 18.7 parts |
| 2-butanone                                                                                                             | 100 parts  |

In this case, the volume ratio of the inorganic pigment (titanium oxide) to the binder resin is 1/1, and the weight ratio of the alkyl resin to the melamine resin is 6/4. The ratio of the particle diameter of the smaller titanium oxide (TTO-F1) to the larger titanium oxide (CR-EL) is 0.16 and the mixing ratio thereof is 1/1.

### Example 23

The procedure for preparation of the photoreceptor in Example 1 was repeated except that the formula of the moiré preventing layer coating liquid was changed as follows.

| Formula of moiré preventing layer coating liquid                                                                   |            |  |
|--------------------------------------------------------------------------------------------------------------------|------------|--|
| Titanium oxide<br>(CR-EL from Ishihara Sangyo Kaisha<br>Ltd., average particle diameter of<br>0.25 $\mu\text{m}$ ) | 42 parts   |  |
| Titanium oxide<br>(A-100 from Ishihara Sangyo Kaisha Ltd.,<br>average particle diameter of 0.15 $\mu\text{m}$ )    | 42 parts   |  |
| Alkyd resin<br>(BEKKOLITE M6401-50-S from<br>Dainippon Ink & Chemicals, Inc.,<br>solid content of 50%)             | 33.6 parts |  |
| Melamine resin<br>(SUPER BEKKAMIN L-121-60 from<br>Dainippon Ink & Chemicals,<br>Inc., solid content of 60%)       | 18.7 parts |  |
| 2-butanone                                                                                                         | 100 parts  |  |

In this case, the volume ratio of the inorganic pigment (titanium oxide) to the binder resin is 1/1, and the weight ratio of the alkyl resin to the melamine resin is 6/4. The ratio of the particle diameter of the smaller titanium oxide (A-100) to the larger titanium oxide (CR-EL) is 0.6 and the mixing ratio thereof is 1/1.

### Evaluation (Evaluation Method 1)

Each of the thus prepared photoreceptors was set in an image forming apparatus having a constitution as illustrated in FIG. 12. The image forming apparatus includes a laser diode which emits light having a wavelength of 780 nm and which serves as the image irradiator; a polygon mirror configured to scan the light for optical writing; a charging roller; and a transfer device including a transfer belt. A running test in which 200,000 images of an original with an image proportion of 6% are continuously reproduced was performed on each photoreceptor using a A-4 size plain paper, followed by production of white solid images and half tone images. The image forming conditions are as follows.

(1) environmental conditions: 22° C. and 55% RH

(2) charging conditions:

DC bias: -950 V

AC bias: 2.0 kV (peak to peak voltage)

1.5 kHz (frequency)

The image qualities of the white solid images and half tone images, i.e., background development, moiré fringes and image density, were checked and the background development was graded into the following four ranks:

◎: excellent

○: good

Δ: slightly bad

X: bad

The results are shown in Table 4.

TABLE 4

| Photoreceptor | Dispersion used | Image qualities        |                                              |
|---------------|-----------------|------------------------|----------------------------------------------|
|               |                 | Background development | Other image qualities                        |
| Ex. 1         | Dispersion 9    | ◎                      | Excellent                                    |
| Ex. 2         | Dispersion 10   | ◎-○                    | Excellent                                    |
| Ex. 3         | Dispersion 11   | ◎-○                    | Excellent                                    |
| Ex. 4         | Dispersion 9    | ◎                      | Good                                         |
| Ex. 5         | Dispersion 9    | ○                      | Good                                         |
| Ex. 6         | Dispersion 9    | ○                      | Slightly low image density                   |
| Ex. 7         | Dispersion 9    | ○                      | Slight background development                |
| Ex. 8         | Dispersion 9    | ○                      | Good                                         |
| Ex. 9         | Dispersion 9    | ○                      | Slight moiré fringes                         |
| Ex. 10        | Dispersion 9    | ○                      | Slight background development                |
| Ex. 11        | Dispersion 9    | ○                      | Slightly low image density                   |
| Ex. 12        | Dispersion 9    | ○                      | Slight background development                |
| Ex. 13        | Dispersion 9    | ○                      | Slightly low image density                   |
| Ex. 14        | Dispersion 9    | ○                      | Excellent                                    |
| Ex. 15        | Dispersion 9    | ○                      | Excellent                                    |
| Ex. 16        | Dispersion 9    | ○                      | Good                                         |
| Ex. 17        | Dispersion 9    | ○                      | Slight background development                |
| Ex. 18        | Dispersion 9    | ○                      | Slightly low image density                   |
| Ex. 19        | Dispersion 9    | ○                      | Extremely excellent                          |
| Ex. 20        | Dispersion 9    | ○                      | Good                                         |
| Ex. 21        | Dispersion 9    | ○                      | Slight moiré fringes                         |
| Ex. 22        | Dispersion 9    | ○                      | Extremely slight moiré fringes               |
| Ex. 23        | Dispersion 9    | ○                      | Good                                         |
| Comp.         | Dispersion 1    | Δ-X                    | Slight background development                |
| Ex. 1         | Dispersion 2    | X                      | Background development                       |
| Ex. 2         | Dispersion 3    | X                      | Background development                       |
| Ex. 3         | Dispersion 4    | X                      | Background development                       |
| Ex. 4         | Dispersion 5    | X                      | Background development                       |
| Comp.         | Dispersion 6    | X                      | Background development                       |
| Ex. 5         | Dispersion 6    | X                      | Background development                       |
| Comp.         | Dispersion 7    | X                      | Background development                       |
| Ex. 6         | Dispersion 7    | X                      | Background development                       |
| Comp.         | Dispersion 8    | X                      | Background development                       |
| Ex. 7         | Dispersion 8    | X                      | Background development                       |
| Comp.         | Dispersion 12   | Δ-X                    | Slight background development                |
| Ex. 8         | Dispersion 12   | X                      | Background development                       |
| Comp.         | Dispersion 13   | X                      | Background development                       |
| Ex. 9         | Dispersion 9    | X                      | Background development, dielectric breakdown |
| Comp.         | Dispersion 9    | ○                      | Moiré fringes                                |
| Ex. 10        | Dispersion 9    | X                      | Background development, dielectric breakdown |
| Comp.         | Dispersion 9    | ○                      | Moiré fringes                                |
| Ex. 11        | Dispersion 9    | X                      | Background development, dielectric breakdown |
| Comp.         | Dispersion 9    | ○                      | Moiré fringes                                |
| Ex. 12        | Dispersion 9    | ○                      | Moiré fringes                                |
| Comp.         | Dispersion 9    | ○                      | Low image density                            |
| Ex. 13        | Dispersion 9    | ○                      | Low image density                            |

### Example 24

The procedure for preparation of the photoreceptor in Example 1 was repeated except that the charge transport layer coating liquid was replaced with the following.

Charge transport polymer having the following formula  
(weight average molecular weight of 135,000)

10 parts



Additive having the following formula

0.5 parts



Methylene chloride

100 parts

## Example 25

35

-continued

Protective layer coating liquid

4 parts

Particulate alumina  
(resistivity of  $2.5 \times 10^{12} \Omega \cdot \text{cm}$ , average primary particle diameter of 0.4  $\mu\text{m}$ )Cyclohexanone 500 parts  
Tetrahydrofuran 150 parts

45

Protective layer coating liquid

Polycarbonate 10 parts  
(TS2050 from Teijin Chemical Ltd., viscosity average molecular weight of 50,000)  
Charge transport material having the following formula 7 parts



50 The procedure for preparation of the photoreceptor in Example 25 was repeated except that the particulate alumina in the protective layer coating liquid was replaced with the following titanium oxide.

55 Titanium oxide 4 parts  
(resistivity of  $1.5 \times 10^{10} \Omega \cdot \text{cm}$ , average primary particle diameter of 0.5  $\mu\text{m}$ )

60

## Example 27

65 The procedure for preparation of the photoreceptor in Example 25 was repeated except that the particulate alumina in the protective layer coating liquid was replaced with the following tin oxide—antimony oxide powder.

Tin oxide - antimony oxide powder  
(resistivity of  $1 \times 10^6 \Omega \cdot \text{cm}$ , average primary  
particle diameter of  $0.4 \mu\text{m}$ )

## Example 28

The procedure for preparation of the photoreceptor in Example 1 was repeated except that the thickness of the charge transport layer was changed to  $18 \mu\text{m}$ , and the following protective layer coating liquid was coated on the charge transport layer, followed by drying to prepare a protective layer having a thickness of  $5 \mu\text{m}$ .

## Protective layer coating liquid

Methyltrimethoxy silane 100 parts  
3% acetic acid 20 parts  
Charge transport material having the following formula 35 parts



Antioxidant 1 part  
(SANOL LS2626 from Sankyo Chemical Co., Ltd.)  
Crosslinking agent (dibutyl tin acetate) 1 part  
2-propanol 200 parts

## Example 29

The procedure for preparation of the photoreceptor in Example 1 was repeated except that the thickness of the charge transport layer was changed to  $18 \mu\text{m}$ , and the following protective layer coating liquid was coated on the charge transport layer, followed by drying to prepare a protective layer having a thickness of  $5 \mu\text{m}$ .

## Protective layer coating liquid

Methyltrimethoxy silane 100 parts  
3% acetic acid 20 parts  
Charge transport material having the following formula 35 parts

-continued

## Protective layer coating liquid

5 HOCH<sub>2</sub>  
10  
15  
10 HOCH<sub>2</sub>  
15 C=CH-  
15 CH<sub>3</sub>  
20 Particulate  $\alpha$ -alumina 15 parts  
(SUMICORUNDUM AA-03 from Sumitomo Chemical Co.,  
Ltd.)  
20 Antioxidant 1 part  
(SANOL LS2626 from Sankyo Chemical Co., Ltd.)  
20 Polycarboxylic acid (BYK P104 from Byk Chemie) 0.4 parts  
Crosslinking agent (dibutyl tin acetate) 1 part  
25 2-propanol 200 parts

## Evaluation (Evaluation Method 2)

30 Each of the thus prepared photoreceptors of Examples  
24-29 and the photoreceptor of Example 1 was set in an  
image forming apparatus having a constitution as illustrated  
in FIG. 12. The image forming apparatus includes a laser  
diode which emits light having a wavelength of  $780 \text{ nm}$  and  
35 which serves as the image irradiator; a polygon mirror  
configured to scan the light for optical writing; and a  
short-range charging roller which has a constitution as  
illustrated in FIG. 13 and which is prepared by winding an  
insulating tape with a thickness of  $50 \mu\text{m}$  on both side  
40 portions of a charging roller (i.e., the gap between the  
surface of the photoreceptor and surface of the charging  
roller is  $50 \mu\text{m}$ ). A running test in which 200,000 images of  
an original with an image proportion of 6% are continuously  
45 reproduced was performed on each photoreceptor using a  
A-4 size plain paper, followed by production of white solid  
images and half tone images. The image forming conditions  
are as follows.

50 (1) environmental conditions:  $22^\circ \text{ C.}$  and 55% RH  
(2) charging conditions:

DC bias:  $-900 \text{ V}$

AC bias: 2.0 kV (peak to peak voltage)

55 2.0 kHz (frequency)

The image qualities of the white solid images and half  
toner images, i.e., background development, moiré fringes  
and image density, were checked and the background develop-  
50 ment was graded into the following four ranks:

60  $\odot$ : excellent

$\circ$ : good

$\Delta$ : slightly bad

X: bad

65 In addition, the abrasion amount of the surface of each  
photoreceptor was measured after the running test.

The results are shown in Table 5.

TABLE 5

| Photoreceptor | Dispersion used | Image qualities        |                         | Abrasion<br>( $\mu\text{m}$ ) |
|---------------|-----------------|------------------------|-------------------------|-------------------------------|
|               |                 | Background development | Half tone image quality |                               |
| Ex. 1         | Dispersion 9    | ◎                      | Good                    | 5.9                           |
| Ex. 24        | Dispersion 9    | ◎                      | Good                    | 3.7                           |
| Ex. 25        | Dispersion 9    | ◎                      | Good                    | 2.5                           |
| Ex. 26        | Dispersion 9    | ◎                      | Good                    | 2.3                           |
| Ex. 27        | Dispersion 9    | ○                      | Slightly blurred        | 2.5                           |
| Ex. 28        | Dispersion 9    | ◎                      | Good                    | 1.9                           |
| Ex. 29        | Dispersion 9    | ◎                      | Good                    | 1.3                           |

## Example 30

The photoreceptor of Example 1 was evaluated by the evaluation method 2 except that after 200,000-sheet running test, half tone images were also produced under environmental conditions of 30° C. and 90% RH to be evaluated.

## Example 31

The procedure for evaluation of the photoreceptor in Example 30 was repeated except that the short-range charger used for the image forming apparatus was replaced with a scorotron charger while the potential of the image area of the photoreceptor was controlled so as to be -900 V.

## Example 32

The procedure for evaluation of the photoreceptor in Example 30 was repeated except that the short-range charger used for the image forming apparatus was replaced with a contact charging roller (i.e., the gap is 0  $\mu\text{m}$ ).

## Example 33

The procedure for evaluation of the photoreceptor in Example 32 was repeated except that the charging conditions were changed to the following.

DC bias: -1600 V (the potential of image area is -900 V)  
AC bias: 0

## Example 34

The procedure for evaluation of the photoreceptor in Example 30 was repeated except that the charging conditions were changed to the following.

DC bias: -1600 V (the potential of image area is -900 V)  
AC bias: 0

## Example 35

The procedure for evaluation of the photoreceptor in Example 30 was repeated except that the gap between the surface of the short-range charger and the surface of the photoreceptor was changed to 70  $\mu\text{m}$ .

## Example 36

The procedure for evaluation of the photoreceptor in Example 30 was repeated except that the gap between the surface of the short-range charger and the surface of the photoreceptor was changed to 100  $\mu\text{m}$ .

## Example 37

The procedure for evaluation of the photoreceptor in Example 30 was repeated except that the gap between the surface of the short-range charger and the surface of the photoreceptor was changed to 150  $\mu\text{m}$ .

## Example 38

10 The photoreceptor of Example 24 was evaluated by the evaluation method 2 except that after 200,000-sheet running test, half tone images were also produced under environmental conditions of 30° C. and 90% RH to be evaluated.

## Example 39

15 The photoreceptor of Example 25 was evaluated by the evaluation method 2 except that after 200,000-sheet running test, half tone images were also produced under environmental conditions of 30° C. and 90% RH to be evaluated.

The evaluation results are shown in Table 6.

TABLE 6

| 25 | Ex. 30 | Image qualities<br>(22° C./55% RH) |                                       |                                       | Note                                                    |
|----|--------|------------------------------------|---------------------------------------|---------------------------------------|---------------------------------------------------------|
|    |        | Background development             | Half tone image                       | Half tone image (30° C./90% RH)       |                                                         |
| 30 | Ex. 30 | ○                                  | Good                                  | Good                                  |                                                         |
| 31 | Ex. 31 | ○                                  | Very slightly blurred                 | Slightly blurred                      | There was strong smell of ozone during the running test |
| 35 | Ex. 32 | ○                                  | Very slightly uneven in image density | Very slightly uneven in image density | The charging roller was soiled.                         |
| 40 | Ex. 33 | ○                                  | Slightly uneven in image density      | Slightly uneven in image density      | The charging roller was soiled.                         |
| 45 | Ex. 34 | ○                                  | Slightly uneven in image density      | Slightly uneven in image density      |                                                         |
| 50 | Ex. 35 | ○                                  | Good                                  | Good                                  |                                                         |
| 55 | Ex. 36 | ○                                  | Good                                  | Good                                  |                                                         |
| 60 | Ex. 37 | ○                                  | Slightly uneven in image density      | Slightly uneven in image density      |                                                         |
| 65 | Ex. 38 | ◎                                  | Good                                  | Good                                  |                                                         |
|    | Ex. 39 | ◎                                  | Good                                  | Good                                  |                                                         |

## Comparative Example 14

55 The procedure for preparation of the photoreceptor in Comparative Example 1 was repeated except that the aluminum cylinder serving as the substrate of the photoreceptor was replaced with an aluminum cylinder having a diameter of 30 mm.

## Comparative Example 15

65 The procedure for preparation of the photoreceptor in Comparative Example 4 was repeated except that the alu-

61

minimum cylinder serving as the substrate of the photoreceptor was replaced with an aluminum cylinder having a diameter of 30 mm.

## Comparative Example 16

The procedure for preparation of the photoreceptor in Comparative Example 5 was repeated except that the aluminum cylinder serving as the substrate of the photoreceptor was replaced with an aluminum cylinder having a diameter of 30 mm.

## Example 40

The procedure for preparation of the photoreceptor in Example 1 was repeated except that the aluminum cylinder serving as the substrate of the photoreceptor was replaced with an aluminum cylinder having a diameter of 30 mm.

## Example 41

The procedure for preparation of the photoreceptor in Example 2 was repeated except that the aluminum cylinder serving as the substrate of the photoreceptor was replaced with an aluminum cylinder having a diameter of 30 mm.

## Comparative Example 17

The procedure for preparation of the photoreceptor in Comparative Example 11 was repeated except that the aluminum cylinder serving as the substrate of the photoreceptor was replaced with an aluminum cylinder having a diameter of 30 mm.

## Comparative Example 18

The procedure for preparation of the photoreceptor in Comparative Example 12 was repeated except that the aluminum cylinder serving as the substrate of the photoreceptor was replaced with an aluminum cylinder having a diameter of 30 mm.

## Comparative Example 19

The procedure for preparation of the photoreceptor in Comparative Example 13 was repeated except that the aluminum cylinder serving as the substrate of the photoreceptor was replaced with an aluminum cylinder having a diameter of 30 mm.

## Evaluation (Evaluation Method 3)

Each of the photoreceptors of Examples 40-41 and Comparative Examples 14-19 was set in each of four process cartridges together with a charger, and the four process cartridges were set in a full color image forming apparatus having the constitution as illustrated in FIG. 16. Then a running test in which 200,000 images of a full color original image are continuously produced was performed under conditions of 22° C. and 55% RH. The charging conditions are as follows.

DC bias: -800 V

AC bias: 1.8 kV (peak to peak voltage)

2.0 kHz (frequency)

Charger: the short-range charger which is the same as that used in the evaluation method 2

Optical writing: laser diode emitting light with wavelength of 780 nm and polygon mirror

Transfer bias: (1) 75 µA and (2) 60 µA (current)

62

After the running test, the color image was observed to determine whether the resultant image has background development and omissions and to evaluate the half tone image qualities.

The image qualities, i.e., background development and omissions, were graded into the following four ranks:

◎: excellent

○: good

Δ: slightly bad

X: bad

The results are shown in Table 7.

TABLE 7

| Photoreceptor | Dispersion used | Image qualities        |                            |
|---------------|-----------------|------------------------|----------------------------|
|               |                 | Background development | Half tone image quality    |
| Ex. 40        | Dispersion 9    | ◎                      | Good                       |
| Ex. 41        | Dispersion 10   | ◎                      | Good                       |
| Comp. Ex. 14  | Dispersion 1    | X                      | Poor color reproducibility |
| Comp. Ex. 15  | Dispersion 4    | X                      | Low image density          |
| Comp. Ex. 16  | Dispersion 5    | X                      | Poor color reproducibility |
| Comp. Ex. 17  | Dispersion 9    | X                      | Poor color reproducibility |
| Comp. Ex. 18  | Dispersion 9    | ○                      | Moiré fringes              |
| Comp. Ex. 19  | Dispersion 9    | ◎                      | Low image density          |

Finally, an experiment was performed to confirm whether the lowest angle peak of the X-ray diffraction spectrum of the titanyl phthalocyanine crystal used for the present invention, which is observed at an angle of 7.3°, is the same as or different from the lowest angle peak of the X-ray diffraction spectrum of known titanyl phthalocyanine crystals, which is observed at an angle of 7.5°.

## Comparative Synthesis Example 9

The procedure for preparation of the titanyl phthalocyanine crystal in Comparative Synthesis Example 1 and the X-ray diffraction analysis was repeated except that the crystal conversion solvent was changed from methylene chloride to 2-butanone. The X-ray diffraction spectrum of the thus prepared titanyl phthalocyanine is illustrated in FIG. 19. As clearly understood from comparison of the X-ray diffraction spectrum of the titanyl phthalocyanine for use in the present invention as shown in FIG. 18 with that of the above-prepared titanyl phthalocyanine as shown in FIG. 19, the lowest angle peak (7.3°) of the titanyl phthalocyanine crystal for use in the present invention is different from the lowest angle peak (7.5°) of the above-prepared titanyl phthalocyanine.

## Measurement Example 1

The titanyl phthalocyanine pigment which was prepared in Comparative Synthesis Example 1 and which has a lowest angle peak at 7.3° was mixed with a titanyl phthalocyanine pigment which was prepared by the same method as disclosed in JP-A 61-239248 and which has a lowest angle peak at 7.5°, in a weight ratio of 100:3. The mixture was mixed in a mortar. The mixture was subjected to the X-ray diffraction analysis. The spectrum of the mixture is shown in FIG. 20.

## Measurement Example 2

The titanyl phthalocyanine pigment which was prepared in Comparative Synthesis Example 9 and which has a lowest angle peak at 7.5° was mixed with a titanyl phthalocyanine pigment which was prepared by the same method as disclosed in JP-A 61-239248 and which has a lowest angle peak at 7.5°, in a weight ratio of 100:3. The mixture was mixed in a mortar. The mixture was subjected to the X-ray diffraction analysis. The spectrum of the mixture is shown in FIG. 21.

As can be understood from the spectrum as shown in FIG. 20, two independent peaks are present at 7.3° and 7.5°. Therefore, the peaks are different from the other. In contrast, in the spectrum as shown in FIG. 21, only one lowest angle peak is present at 7.5°, namely the spectrum as shown in FIG. 21 is clearly different from the spectrum as shown in FIG. 20. Therefore, the lowest angle peak (7.3°) of the titanyl phthalocyanine pigment of is clearly different from the lowest angle peak (7.5°) of the conventional titanyl phthalocyanine pigment.

## Effects of the Present Invention

By using the photoreceptor of the present invention, high quality images can be stably produced without causing abnormal images. Specifically, the photoreceptor of the present invention hardly causes the problems in that background development is caused after long repeated use; residual potential increases; and dielectric break down which causes omissions in the resultant images occurs when a contact charger or a short-range charger is used for charging the photoreceptor.

The image forming apparatus of the present invention which includes the photoreceptor of the present invention can stably produce high quality images for a long period of time with hardly causing abnormal images. Specifically, problems specific to the nega-posi development method such as occurrence of background development and decrease of image density can be avoided.

In addition, the process cartridge of the present invention including the photoreceptor of the present invention can produce high quality images while having good durability.

This document claims priority and contains subject matter related to Japanese Patent Applications No. 2003-342515, and 2003-401588, filed on Sep. 30, 2003, and Dec. 1, 2003, respectively, incorporated herein by reference.

Having now fully described the invention, it will be apparent to one of ordinary skill in the art that many changes and modifications can be made thereto without departing from the spirit and scope of the invention as set forth therein.

What is claimed as new and desired to be secured by Letters Patent of the United States is:

1. A photoreceptor, comprising:  
an electroconductive cylindrical metal substrate;  
a charge blocking layer located overlying and directly contacting the electroconductive cylindrical metal substrate, wherein the charge blocking layer includes a polyamide and has a thickness of less than 2.0  $\mu\text{m}$ ;  
a moiré preventing layer located overlying and directly contacting the charge blocking layer, wherein the moiré preventing layer includes titanium oxide and a thermosetting resin including an alkyd resin and a melamine resin, and wherein a volume ratio of the titanium oxide to the thermosetting resin is from 1/1 to 3/1 and a weight ratio of the alkyd resin to the melamine resin is from 5/5 to 8/2; and

a photosensitive layer located overlying and directly contacting the moiré preventing layer, wherein the photosensitive layer comprises a titanyl phthalocyanine crystal which has an average primary particle diameter not greater than 0.25  $\mu\text{m}$ , and has a first X-ray diffraction spectrum such that a maximum peak is observed at a Bragg (20) angle of 27.2° $\pm$ 0.2°; a peak is observed at Bragg (20) angle of 9.4° $\pm$ 0.2°, 9.6 $\pm$ 0.2° and 24.0 $\pm$ 0.2°; a lowest angle peak is observed at an angle of 73° $\pm$ 0.2°; no peak is observed between the lowest angle peak and the 9.4° peak; and no peak is observed at a Bragg (20) angle of 26.3° $\pm$ 0.2°, when a Cu-K $\alpha$  X-ray having a wavelength of 0.1542 nm (1.542  $\text{\AA}$ ) is used.

2. The photoreceptor according to claim 1, wherein the photosensitive layer comprises a charge generation layer including the titanyl phthalocyanine crystal and a charge transport layer, which are overlaid.

3. The photoreceptor according to claim 1, wherein the photosensitive layer is prepared by a method comprising:  
providing a coating liquid which includes at least the titanyl phthalocyanine crystal and a solvent and in which the titanyl phthalocyanine crystal is dispersed in the solvent while having a particle diameter distribution such that an average particle diameter is not greater than 0.3  $\mu\text{m}$  and a standard deviation is not greater than 0.2  $\mu\text{m}$ ;  
filtering the coating liquid using a filter having an effective pore diameter not greater than 3  $\mu\text{m}$ ;  
coating the coating liquid overlying the moiré preventing layer; and drying the coated liquid.

4. The photoreceptor according to claim 1, wherein the titanyl phthalocyanine crystal is prepared by a method comprising:

providing a titanyl phthalocyanine raw material which has either one of an amorphous state or a low crystallinity and which has an average particle diameter not greater than 0.1  $\mu\text{m}$  and has a second X-ray diffraction spectrum such that a maximum peak having a half width not less than 1° is observed at a Bragg (20) angle of from 7.0° to 7.5° with a tolerance of  $\pm$ 0.2°;  
changing a crystal form of the titanyl phthalocyanine raw material in an organic solvent in the presence of water to prepare the titanyl phthalocyanine crystal having the first X-ray diffraction spectrum; and  
filtering the dispersion including the titanyl phthalocyanine crystal before the average primary particle diameter exceeds 0.25  $\mu\text{m}$ .

5. The photoreceptor according to claim 4, wherein the titanyl phthalocyanine raw material providing step comprising:

providing the titanyl phthalocyanine raw material by an acid paste method; and  
then washing the titanyl phthalocyanine raw material using ion-exchange water to an extent such that the ion-exchange water used for washing have at least one of a pH of from 6 to 8 and a specific conductivity not greater than 8.

6. The photoreceptor according to claim 4, wherein an amount of the organic solvent used in the crystal changing step is not less than 30 times that of the titanyl phthalocyanine raw material.

7. The photoreceptor according to claim 1, wherein the titanyl phthalocyanine crystal is synthesized using raw materials including no halogen atom.

8. The photoreceptor according to claim 1, wherein the titanium oxide comprises a titanium oxide (T1) having an average particle diameter of D1, and another titanium oxide

## 65

(T2) having an average particle diameter of D2, and wherein the following relationship is satisfied:

$$0.2 < (D2/D1) \leq 0.5.$$

9. The photoreceptor according to claim 8, wherein the average particle diameter D2 is greater than 0.05  $\mu\text{m}$  and less than 0.2  $\mu\text{m}$ . 5

10. The photoreceptor according to claim 8, wherein the titanium oxide T1 and the titanium oxide T2 are included in a weight ratio such that the following relationship is satisfied:

$$0.2 \leq T2/(T1+T2) \leq 0.8.$$

11. The photoreceptor according to claim 1, further comprising a protective layer located overlying the photosensitive layer. 15

12. The receptor according to claim 11, further comprising a protective layer comprises an inorganic pigment having a resistivity not less than  $10^{10} \Omega\cdot\text{cm}$ .

13. The photoreceptor according to claim 12, wherein the inorganic pigment is a material selected from the group 20 consisting of alumina, titanium oxide and silica.

14. The photoreceptor according to claim 13, wherein the inorganic pigment is  $\alpha$ -alumina.

15. The photoreceptor according to claim 11, wherein the protective layer comprises a charge transport polymer.

16. The photoreceptor according to claim 11, wherein the protective layer comprises a crosslinked resin. 25

17. The photoreceptor according to claim 16, wherein the crosslinked resin has a charge transport moiety therein.

18. A method for manufacturing the photoreceptor according to claim 2, comprising forming the charge blocking layer overlying the electroconductive substrate:

forming the moire preventing layer overlying the charge blocking layer;

forming the charge generation layer overlying the moire preventing layer; and

forming the charge transport layer overlying the charge generation layer,

wherein the charge generation layer forming step includes:

providing a titanyl phthalocyanine raw material having either one of an amorphous state and a low crystallinity and which has an average particle diameter not greater than 0.1  $\mu\text{m}$  and has a second X-ray diffraction spectrum such that a maximum peak having a half width not less than  $1^\circ$  is observed at a Bragg (20) angle of from  $7.0^\circ$  to  $7.5^\circ$  with a tolerance of  $\pm 0.2^\circ$ ;

changing a crystal form of the titanyl phthalocyanine raw material in an organic solvent in the presence of water to prepare the titanyl phthalocyanine crystal having the first X-ray diffraction spectrum;

filtering the dispersion including the crystal-changed titanyl phthalocyanine crystal before the average primary particle diameter exceeds 0.25  $\mu\text{m}$ ;

providing a coating liquid which includes at least the titanyl phthalocyanine crystal and a solvent and in which the titanyl phthalocyanine crystal is dispersed in the solvent while having a particle diameter distribution such that an average particle diameter is not greater than 0.3  $\mu\text{m}$  and a standard deviation is not greater than 0.2  $\mu\text{m}$ ;

filtering the coating liquid using a filter having an effective pore diameter not greater than 3  $\mu\text{m}$ ;

coating the coating liquid overlying the moire preventing layer; and drying the coated liquid.

19. The method according to claim 18, wherein the titanyl phthalocyanine raw material having either one of an amorphous state or a low crystallinity is prepared by a method comprising:

## 66

providing a crude titanyl phthalocyanine; subjecting the crude titanyl phthalocyanine to an acid paste treatment to prepare the titanyl phthalocyanine raw material; and then

washing the titanyl phthalocyanine raw material using ion-exchange water to an extent such that the ion-exchange water used for washing have at least one of a pH of from 6 to 8 and a specific conductivity not greater than 8.

20. The method according to claim 18, wherein an amount of the organic solvent used in the crystal changing step is not less than 30 times that of the titanyl phthalocyanine raw material.

21. The method according to claim 20, wherein the crude titanyl phthalocyanine crystal is synthesized using raw materials including no halogen atom.

22. An image forming apparatus comprising:  
at least one image forming unit comprising:  
the photoreceptor according to claim 1;  
a charger configured to charge the photoreceptor;  
a light irradiator configured to irradiate the photoreceptor with imagewise light to form an electrostatic latent image on the photoreceptor;

a developing device configured to develop the electrostatic latent image with a developer including a toner to form a toner image on the photoreceptor; and

a transfer device configured to transfer the toner image onto a receiving material optionally via an intermediate transfer medium, and

a fixer configured to fix the toner image on the receiving material.

23. The image forming apparatus according to claim 22, 35 wherein the image forming apparatus includes two or more of the image forming units.

24. The image forming apparatus according to claim 22, wherein the charger is one of a contact charger and a short-range charger which charges the photoreceptor while a gap is formed between a surface of the charger and a 40 surface of the photoreceptor.

25. The image forming apparatus according to claim 24, wherein the charger is a short-range charger, and wherein the gap is not greater than 100  $\mu\text{m}$ .

26. The image forming apparatus according to claim 22, wherein the charger applies a DC voltage overlapped with an AC voltage.

27. The image forming apparatus according to claim 22, 50 wherein the at least one image forming unit further comprises a cleaner configured to clean a surface of the photoreceptor, and wherein the photoreceptor, and at least one of the light irradiator, the developing device and the cleaner form a cartridge which is detachably set in the image forming apparatus.

28. A process cartridge comprising:  
the photoreceptor according to claim 1; and  
at least a device selected from the group consisting of a charger configured to charge the photoreceptor; a light irradiator configured to irradiate the photoreceptor with imagewise light to form an electrostatic latent image on the photoreceptor; a developing device configured to develop the electrostatic latent image with a developer including a toner to form a toner image on the photoreceptor; and a cleaner configured to clean a surface of the photoreceptor.